# EUROPEAN PATENT APPLICATION

(11) **EP 2 463 717 A1**
(43) Date of publication of application: **13.06.2012**
(21) Application number: 10806518.6
(22) Date of filing: 05.08.2010
(51) Int. Cl.: G03G 9/097, G03G 9/087

(54) **POLYMERIZED TONER COMPRISING CYCLIC PHENOL SULFIDE**

(30) Priority: 07.08.2009 JP 2009184019
(71) Applicant: Hodogaya Chemical Co., Ltd., Tokyo 105-0011 (JP)
(72) Inventor: YASUMURA Masateru, Shunan-shi Yamaguchi 746-0042 (JP); ITO Masami, Tsukuba-shi Ibaraki 305-0841 (JP); TSUJI Motonori, Tsukuba-shi Ibaraki 305-0841 (JP); TOJOU Masaya, Tsukuba-shi Ibaraki 305-0841 (JP); SAWANO Masataka, Tokyo, 105-0011 (JP); HIRAISHI Kanae, Fukushima 963-8802 (JP)
(74) Representative: Eisenführ, Speiser & Partner
(86) International application number: PCT/JP2010/063295
(87) International publication number: WO 2011/016519

(57) **Abstract**

The present invention discloses a negatively charged polymerized toner having high charging performance which comprises a charge control agent particularly useful for color toners and polymerized toners, said charge control agent comprising a cyclic phenol sulfide(s) as an active ingredient which speeds up charging risetime, has a high charge amount and charging characteristics particularly excellent in environmental stability, and is safe since it does not have any problem with the waste regulations.

Namely, the present invention discloses a polymerized toner comprising one or more kinds of a cyclic phenol sulfide(s) of the following formula (1): wherein R1 is a substituted or unsubstituted and straight or branched alkyl group having 1 to 20 carbon atoms, a substituted or unsubstituted aromatic hydrocarbon group, or a substituted or unsubstituted condensed polycyclic aromatic group; R2 is a substituted or unsubstituted and straight or branched alkyl group having 1 to 20 carbon atoms, a substituted or unsubstituted aromatic hydrocarbon group, a substituted or unsubstituted aromatic heterocyclic group, or a substituted or unsubstituted condensed polycyclic aromatic group; m is an integer from 4 to 9; and n is an integer of 0, 1 or 2.

## Description

### Technical Field of the Invention

The present invention relates to negatively charged polymerized toners containing charge control agents used in an image forming apparatus which visualizes electrostatic latent images in electrophotography, the electrostatic recording and the like.

### Background of the Invention

In the image forming process according to electrophotography, electrostatic latent images are formed on the inorganic photoreceptor such as selenium, selenium alloy, cadmium sulfide and amorphous silicon or on the organic photoreceptor using a charge generator and a charge transporting agent. Then, the images are developed by a toner, transferred to paper, plastic film or the like and fixed to obtain visible images.

As for photoreceptors, depending on the composition thereof, there are photoreceptors having a positive charge and those having a negative charge. In the case of forming printing parts as electrostatic latent images by exposure, the images are developed by a toner of the opposite sign electrical charge. On the other hand, in the case of reversely developing printing parts by removing the electricity thereof, the images are developed by a toner of the same sign electrical charge. A toner comprises a binder resin, a coloring agent and other additives, and a charge control agent is usually used therein in order to provide desired frictional charge characteristics such as charge speed, charge level, and charge stability, temporal stability, and environmental stability. The charge control agent largely affects the characteristics of a toner.

Further, in the case of color toners, a light-colored and preferably colorless charge control agent is needed, which does not affect the hue. Examples of such light-colored or colorless charge control agents include metal complex salt compounds of hydroxybenzoic acid derivatives (see Patent Literatures 1 to 3), metal salt compounds of aromatic dicarboxylic acids (see Patent Literature 4), metal complex salt compounds of anthranilic acid derivatives (see Patent Literatures 5 and 6), organic boron compounds (see Patent Literatures 7 and 8), biphenol compounds (see Patent Literature 9), calyx(n)arene compounds (see Patent Literatures 10 to 15), and cyclic phenol sulfides (see Patent Literatures 16 to 18) for a negatively charged toner; and quaternary ammonium salt compounds (see Patent Literatures 19 to 23) for a positively charged toner.

A toner mainly used until now is a crushed toner produced by crushing and powderizing pigments. Since such crushed toner does not have a uniform particle form or size, it easily produces differences in electrical characteristics when transferring the images on a photoconductive drum or paper. Therefore, in order to solve the above problem of a crushed toner, a higher-quality polymerized toner is proposed (see Patent Literature 24: The description of this literature is included in the description of the present specification). In this polymerized toner, particles of the toner are produced by binding binder resins which are polymers in a chemical reaction using a liquid medium. The particles of thus produced polymerized toner are spherical, and size thereof is uniform and small. Therefore, gradation quality of the toner can be enhanced by increasing resolution, and as a result, higher image quality can be achieved. Generally, a polymerized toner is produced by emulsion polymerization or suspension polymerization.

Under the above circumstances, when using a publicly known charge control agent in a polymerized toner, many of the charge control agents are complexes or salts which comprise metals such as chromium and zinc, and not always safe since they have a problem with the waste regulations. In addition, such charge control agents are disadvantageous in that they cannot be completely colorless; they are late in charging risetime; they have a problem with the environmental stability of the charge amount in hot and humid conditions; the charge amount thereof is low; oppositely-charged toners are numerously generated; or they are poor in dispersibility or stability of the compound. Further, some of them cannot be applied to a polymerized toner. Thus, there has been no compound having satisfactory performance as a charge control agent for a polymerized toner.
- Patent Literature 1:: JP-B 55-042752
- Patent Literature 2:: JP-A 61-069073
- Patent Literature 3:: JP-A 61-221756
- Patent Literature 4:: JP-A 57-111541
- Patent Literature 5:: JP-A 61-141453
- Patent Literature 6:: JP-A 62-094856
- Patent Literature 7:: US-A 4767688
- Patent Literature 8:: JP-A 1-306861
- Patent Literature 9:: JP-A 61-003149
- Patent Literature 10:: JP-B 2568675
- Patent Literature 11:: JP-B 2899038
- Patent Literature 12:: JP-B 3359657
- Patent Literature 13:: JP-B 3313871
- Patent Literature 14:: JP-B 3325730
- Patent Literature 15:: JP-A 2003-162100
- Patent Literature 16:: JP-A 2003-295522
- Patent Literature 17:: WO 2007/111346
- Patent Literature 18:: WO 2007/119797
- Patent Literature 19:: JP-A 57-119364
- Patent Literature 20:: JP-A 58-009154
- Patent Literature 21:: JP-A 58-098742
- Patent Literature 22:: JP-A 10-081680
- Patent Literature 23:: WO 98/09959
- Patent Literature 24:: JP-A 2008-165017

### Disclosure of the Invention

The object of the present invention is to provide novel cyclic phenol sulfides. The further object of the present invention is, in the light of the above circumstances, to provide charge control agents particularly useful for color toners and polymerized toners, which speed up charging risetime, have a high charge amount and charging characteristics particularly excellent in environmental stability, and are safe since they do not have any problem with the waste regulations. The additional object of the present invention is to provide negatively charged polymerized toners having high charging performance which comprise said charge control agents.

The present invention has been completed by the thorough research to achieve the above objects. Namely, the present invention provides the followings.
1. A polymerized toner comprising one or more kinds of a cyclic phenol sulfide(s) of the following formula (1): wherein R1 is a substituted or unsubstituted and straight or branched alkyl group having 1 to 20 carbon atoms, a substituted or unsubstituted aromatic hydrocarbon group, or a substituted or unsubstituted condensed polycyclic aromatic group; R2 is a substituted or unsubstituted and straight or branched alkyl group having 1 to 20 carbon atoms, a substituted or unsubstituted aromatic hydrocarbon group, a substituted or unsubstituted aromatic heterocyclic group, or a substituted or unsubstituted condensed polycyclic aromatic group; m is an integer from 4 to 9; and n is an integer of 0, 1 or 2.
2. The polymerized toner according to above 1, wherein, in the formula (1), R2 is a substituted or unsubstituted aromatic hydrocarbon group, a substituted or unsubstituted aromatic heterocyclic group, or a substituted or unsubstituted condensed polycyclic aromatic group.
3. The polymerized toner according to above 1 or 2, wherein, in the formula (1), R2 is an aromatic hydrocarbon group with a substituent(s), a substituted or unsubstituted aromatic heterocyclic group, or a condensed polycyclic aromatic group with a substituent(s).
4. The polymerized toner according to any one of above 1 to 3, wherein, in the formula (1), R2 is a substituted or unsubstituted aromatic heterocyclic group.
5. The polymerized toner according to any one of above 1 to 4 comprising one or more kinds of the cyclic phenol sulfide(s) of the above formula (1), wherein m is 4 or 8; and n is 2.
6. The polymerized toner according to above 1 comprising a charge control agent containing one or more kinds of the cyclic phenol sulfide(s) of the above formula (1) as an active ingredient.
7. The polymerized toner according to above 1 comprising a coloring agent, a binder resin, and a charge control agent containing one or more kinds of the cyclic phenol sulfide(s) of the above formula (1) as an active ingredient.

Examples of straight or branched alkyl groups having 1 to 20 carbon atoms in "a substituted or unsubstituted and straight or branched alkyl group having 1 to 20 carbon atoms" represented by R1 and R2 in the formula (1) include a methyl group, ethyl group, n-propyl group, 2-propyl group, n-butyl group, sec-butyl group, 2-methylpropyl group, tert-butyl group, n-pentyl group, 1-methylbutyl group, 1-ethylpropyl group, 1,1-dimethylpropyl group, 1,2-dimethylpropyl group, n-hexyl group, 1-methylpentyl group, 2-methylpentyl group, 3-methylpentyl group, 4-methylpentyl group, 1-ethylbutyl group, 2-ethylbutyl group, 1,1-dimethylbutyl group, 1,2-dimethylbutyl group, 1,3-dimethylbutyl group, 1,4-dimethylbutyl group, 2,2-dimethylbutyl group, 2,3-dimethylbutyl group, 3,3-dimethylbutyl group, 1-ethyl-2-methyl-propyl group, 1,1,2-trimethylpropyl group, n-heptyl group, 2-methylhexyl group, n-octyl group, isooctyl group, tert-octyl group, 2-ethylhexyl group, 3-methylheptyl group, n-nonyl group, isononyl group, 1-methyloctyl group, 2-ethylheptyl group, n-decyl group, 1-methylnonyl group, n-undecyl group, 1,1-dimethylnonyl group, n-dodecyl group, n-tetradecyl group, n-heptadecyl group, and n-octadecyl group.

Examples of substituents in "a substituted or unsubstituted and straight or branched alkyl group having 1 to 20 carbon atoms" represented by R1 and R2 in the formula (1) include a fluorine atom, chlorine atom, cyano group, hydroxyl group, nitro group, cyclopentyl group, cyclohexyl group, straight or branched alkoxy group having 1 to 6 carbon atoms, dialkylamino group substituted with a straight or branched alkyl group(s) having 1 to 6 carbon atoms, straight or branched acyl group having 1 to 20 carbon atoms, straight or branched alkoxycarbonyl group having 1 to 20 carbon atoms, epoxyalkyl group having 1 to 6 carbon atoms, phenyl group, naphthyl group, anthryl group, fluorenyl group, styryl group, pyridyl group, pyridoindolyl group, quinolyl group, and benzothiazolyl group. These substitutents can be further substituted.

Examples of aromatic hydrocarbon groups in "a substituted or unsubstituted aromatic hydrocarbon group" and condensed polycyclic aromatic groups in "a substituted or unsubstituted condensed polycyclic aromatic group" each represented by R1 in the formula (1) include a phenyl group, biphenyl group, terphenyl group, naphthyl group, anthryl group, phenanthryl group, fluorenyl group, indenyl group, and pyrenyl group.

Examples of substituents in a substituted aromatic hydrocarbon group or a substituted condensed polycyclic aromatic group each represented by R1 in the formula (1) include a fluorine atom, chlorine atom, cyano group, hydroxyl group, nitro group, straight or branched alkyl group having 1 to 6 carbon atoms, cyclopentyl group, cyclohexyl group, straight or branched alkoxy group having 1 to 6 carbon atoms, dialkylamino group substituted with a straight or branched alkyl group(s) having 1 to 6 carbon atoms, phenyl group, naphthyl group, anthryl group, fluorenyl group, styryl group, pyridyl group, pyridoindolyl group, quinolyl group, and benzothiazolyl group. These substitutents can be further substituted.

R1 in the formula (1) is preferably an alkyl group having 1 to 20 carbon atoms, and particularly preferably an alkyl group having 1 to 18 carbon atoms. R1 is also preferably a phenylalkyl group wherein the above alkyl group has a phenyl group as a substituent. Examples of such phenylalkyl groups include a phenylalkyl group wherein an alkyl group such as a benzyl group has 1 to 6 carbon atoms, and more preferably has 1 to 3 carbon atoms.

Examples of aromatic hydrocarbon groups in "a substituted or unsubstituted aromatic hydrocarbon group", aromatic heterocyclic groups in "a substituted or unsubstituted aromatic heterocyclic group" and condensed polycyclic aromatic groups in "a substituted or unsubstituted condensed polycyclic aromatic group" each represented by R2 in the formula (1) include a phenyl group, biphenyl group, terphenyl group, naphthyl group, anthryl group, phenanthryl group, fluorenyl group, indenyl group, pyrenyl group, pyridyl group, triazyl group, pyrimidyl group, furanyl group, pyranyl group, thiophenyl group, quinolyl group, isoquinolyl group, benzofuranyl group, benzothiophenyl group, indolyl group, carbazolyl group, benzooxazolyl group, benzothiazolyl group, quinoxalyl group, benzoimidazolyl group, pyrazolyl group, dibenzofuranyl group, dibenzothiophenyl group, naphthyridinyl group, phenanthrolinyl group, and acridinyl group.

Examples of substituents in a substituted aromatic hydrocarbon group, a substituted aromatic heterocyclic group or a substituted condensed polycyclic aromatic group each represented by R2 in the formula (1) include a fluorine atom, chlorine atom, cyano group, hydroxyl group, nitro group, straight or branched alkyl group having 1 to 6 carbon atoms, cyclopentyl group, cyclohexyl group, straight or branched alkoxy group having 1 to 6 carbon atoms, dialkylamino group substituted with a straight or branched alkyl group(s) having 1 to 6 carbon atoms, phenyl group, naphthyl group, anthryl group, fluorenyl group, styryl group, pyridyl group, pyridoindolyl group, quinolyl group, and benzothiazolyl group. These substitutents can be further substituted.

R2 in the formula (1) is preferably an alkyl group having 1 to 20 carbon atoms, and particularly preferably a branched alkyl group having 3 to 18 carbon atoms. Among them, R2 is particularly preferably a branched alkyl group having 4 to 12 carbon atoms such as a tert-butyl group having a tertiary alkyl group on the terminal thereof.

"n" in the formula (1) is 1 or 2, and n of each molecules may be the same or different from each other. It is preferable that each molecule satisfies 1.5m≦N≦2m when defining a total of n as N. Further preferable range of N is 1.7m≦N≦2m.

"m" in the formula (1) is preferably 4 and/or 8, and particularly preferably 4.

Since the sodium content in the product of a cyclic phenol sulfide of the formula (1) used in the present invention is 1000ppm or less, a toner comprising this cyclic phenol sulfide as an active ingredient wherein the sodium content in the product is 1000ppm or less instantly keeps an appropriate charge (time constant is small) as compared with a conventional toner which comprises a cyclic phenol sulfide having the sodium content in the product beyond 1000ppm as an active ingredient. Thus, the toner comprising the cyclic phenol sulfide of the formula (1) of the present invention has superiority in environmental stability, especially the superiority in that charge does not lower in hot and humid conditions.

As causes making the sodium content in products larger, it is thought that inorganic salts mainly containing sodium get mixed in products in the production process, for example. It is assumed that the sodium content measured in the present invention includes those produced by all of the above causes. The sodium content can be measured by the usual measurement method, namely, by fluorescent X-ray analysis, atomic absorption analysis, ICP emission spectrometry, ICP-MS measurement, analysis with ion chromatography, or the like. In terms of ease of use, fluorescent X-ray analysis is preferable among them.

A charge control agent is defined as a substance which gives stable static charge to a toner. However, when there is a certain amount or more of inorganic salts which are generated as reactant by-products or unreacted organic salts in the cyclic phenol sulfide, the effect of such salts cannot be ignored in humidity environment, and image stability is lacked not only in high humidity environment but also in normal humidity environment when running the toner for a long period.

It is possible to determine salts in a charge control agent by measuring the electrical conductivity thereof when dispersing it in water. However, since some organic salts are hardly soluble in water, precise contents thereof cannot sometimes be calculated.

In the present invention, it has become possible to provide a charge control agent which expresses excellent charging performance and a toner comprising said charge control agent by directly measuring sodium contained in a cyclic phenol sulfide and controlling the sodium content thereof within a certain range.

The charge control agent of the present invention is excellent in the charge control characteristics, the environment resistance and durability. When using it for a polymerized toner, it does not induce fogging and it is possible to obtain images with clear image density, high dot reproducibility and high fine line reproducibility

In the present invention, the charge control agent comprising one or more kinds of a cyclic phenol sulfide(s) of the formula (1) as an active ingredient has a quicker charging risetime, a higher charge amount and charging characteristics particularly excellent in the environmental stability than conventional charge control agents. Further, it is most suitable for color toners and particularly for polymerized toners because it is completely colorless, and it does not contain metals such as chromium and zinc which are concern for the environmental problem. Besides, it is excellent in dispersibility and stability of the compound.

### Best Mode for Carrying out the Invention

A cyclic phenol sulfide of the formula (1) used in the present invention can be produced by conducting publicly known cyclization or oxidization (see Patent Literatures 22 and 23) following the cyclization to a corresponding phenol derivative(s) to produce a corresponding cyclic phenol sulfide, and then conducting publicly known O-alkylation or the like to said cyclic phenol sulfide. It can also be produced by conducting cross-coupling reaction such as Suzuki Coupling to a corresponding cyclic phenol sulfide.

In the present invention, it is preferable to adjust the volume average particle diameter of a charge control agent to 0.1 to 20µm for use, and particularly preferably 0.1 to 10µm. When the volume average particle diameter is smaller than 0.1µm, the charge control agent appearing on the toner surface becomes little and the desired charge control effect cannot be obtained. When the volume average particle diameter is bigger than 20µ m, the charge control agent dropping from the toner increases and the adverse effects such as contamination in the machine occur.

Further, when using a charge control agent in a toner of the present invention, it is preferable to adjust the volume average particle diameter thereof to 1.0µm or smaller for use, and particularly preferably 0.01 to 1.0 µm. When the volume average particle diameter is beyond 1.0µm, the finally obtained particle size distribution of a toner for electrophotography becomes wide, or free grains occur and it sometimes induces performance or reliability degradation. On the other hand, when the volume average particle diameter is within the above range, the above problems do not occur. In addition to it, the maldistribution between toners decreases and dispersibility in the toner becomes better, and therefore, it is advantageous in that differences in performance or reliability become smaller.

Examples of the method of making the cyclic phenol sulfide of the formula (1) which is a charge control agent used in the present invention contained in a toner include the method comprising the steps of adding it to a binder resin together with a coloring agent and the like, kneading, and crushing them (crushed toner); and the method comprising the steps of adding the cyclic phenol sulfide of the formula (1) to polymerizable monomers and polymerizing them to obtain the toner (polymerized toner). Thus, there are the method of adding the cyclic phenol sulfide to the inside of the toner particles in advance (the internal addition) and the method of adding it to the surface of the toner particles which have been produced in advance (the external addition). In the case of internally adding the cyclic phenol sulfide to the toner particles, the preferable additive amount thereof is 0.1 to 10 parts by weight to 100 parts by weight of a binder resin, and more preferably 0.2 to 5 parts by weight. In the case of externally adding the cyclic phenol sulfide to the toner particles, the preferable additive amount thereof is 0.01 to 5 parts by weight to 100 parts by weight of a binder resin and more preferably 0.01 to 2 parts by weight. Further, it is mechanochemically preferable to fix the cyclic phenol sulfide to the surface of the toner particles.

In the present invention, the charge control agent which comprises the cyclic phenol sulfide of the formula (1) as the active ingredient can be combined with the other known charge control agent(s) having a negative charge. Examples of the preferable combined charge control agents include azo iron complexes or complex salts, azo chromium complexes or complex salts, azo manganese complexes or complex salts, azo cobalt complexes or complex salts, azo zirconium complexes or complex salts, chromium complexes or complex salts of carboxylic acid derivatives, zinc complexes or complex salts of carboxylic acid derivatives, aluminum complexes or complex salts of carboxylic acid derivatives, and zirconium complexes or complex salts of carboxylic acid derivatives. The carboxylic acid derivatives are preferably aromatic hydroxyl carboxylic acids, and more preferably 3,5-di-tert-butyl salicylic acid. In addition, the examples include boron complexes or complex salts, and negative resin charge control agents.

In the present invention, in the case of combining the charge control agent with the other charge control agent(s), the preferable additive amount of the charge control agent(s) other than the charge control agent which is the cyclic phenol sulfide of the present invention is 0.1 to 10 parts by weight to 100 parts by weight of a binder resin.

As for the kind of the binder resins used in the toner of the present invention, any publicly known one can be used as the binder resin. Examples thereof include vinyl polymers such as styrene monomers, acrylate monomers and methacrylate monomers or the copolymers comprising two or more kinds of these monomers, polyester resins, (meth)acrylic resins, polyol resins, phenol resins, silicone resins, polyurethane resins, polyamide resins, furan resins, epoxy resins, xylene resins, terpene resins, coumarone-indene resins, polycarbonate resins and petroleum resins. Polyester resins are preferable among them.

Examples of the styrene monomers, acrylate monomers and methacrylate monomers each of which form the vinyl polymers or the copolymers include the followings but not limited to them.

Examples of the styrene monomers are styrenes or derivatives thereof such as styrene, o-methylstyrene, m-methylstyrene, p-methylstyrene, p-phenylstyrene, p-ethylstyrene, 2,4-dimethylstyrene, p-n-amylstyrene, p-tert-butylstyrene, p-n-hexylstyrene, p-n-octylstyrene, p-n-nonylstyrene, p-n-decylstyrene, p-n-dodecylstyrene, p-methoxystyrene, p-chlorostyrene, 3,4-dichlorostyrene, m-nitrostyrene, o-nitrostyrene and p-nitrostyrene.

Examples of the acrylate monomers are acrylic acids or esters thereof such as acrylic acids, methyl acrylate, ethyl acrylate, propyl acrylate, n-butyl acrylate, isobutyl acrylate, n-octyl acrylate, n-dodecyl acrylate, 2-ethylhexyl acrylate, stearyl acrylate, 2-chloroethyl acrylate and phenyl acrylate.

Examples of the methacrylate monomers are methacrylic acids or esters thereof such as methacrylic acids, methyl methacrylate, ethyl methacrylate, propyl methacrylate, n-butyl methacrylate, isobutyl methacrylate, n-octyl methacrylate, n-dodecyl methacrylate, 2-ethylhexyl methacrylate, stearyl methacrylate, phenyl methacrylate, dimethylaminoethyl methacrylate and diethylaminoethyl methacrylate.

Examples of other monomers which form the vinyl polymers or the copolymers include following (1) to (18): (1) monoolefins such as ethylene, propylene, butylene and isobutylene; (2) polyenes such as butadiene and isoprene; (3) vinyl halides such as vinyl chloride, vinylidene chloride, vinyl bromide and vinyl fluoride; (4) vinyl esters such as vinyl acetate, vinyl propionate and vinyl benzoate; (5) vinyl ethers such as vinyl methyl ether, vinyl ethyl ether and vinyl isobutyl ether; (6) vinyl ketones such as methyl vinyl ketone, hexyl vinyl ketone and methyl isopropenyl ketone; (7) N-vinyl compounds such as N-vinylpyrrole, N-vinylcarbazole, N-vinylindole and N-vinylpyrrolidone; (8) vinylnaphthalenes; (9) acrylic acid or methacrylic acid derivatives such as acrylonitrile, methacrylonitrile and acrylamide; (10) unsaturated dibasic acids such as a maleic acid, citraconic acid, itaconic acid, alkenyl succinic acid, fumaric acid and mesaconic acid; (11) unsaturated dibasic acid anhydrides such as maleic anhydride, citraconic anhydride, itaconic anhydride and alkenyl succinic anhydride; (12) monoesters of unsaturated dibasic acids such as maleic acid monomethylester, maleic acid monoethylester, maleic acid monobutylester, citraconic acid monomethylester, citraconic acid monoethylester, citraconic acid monobutylester, itaconic acid monomethylester, alkenyl succinic acid monomethylester, furamic acid monomethylester and mesaconic acid monomethylester; (13) unsaturated dibasic acid esters such as dimethyl maleate and dimethyl fumarate; (14) α,β-unsaturated acids such as a crotonic acid and cinnamic acid; (15) α,β-unsaturated acid anhydrides such as crotonic anhydride and cinnamic anhydride; (16) monomers having a carboxyl group(s) such as anhydrides of the α,β-unsaturated acid and lower fatty acids, an alkenyl malonic acid, alkenyl glutaric acid, alkenyl adipic acid, and acid anhydrides and monoesters thereof; (17) hydroxyalkyl esters of acrylic acids or methacrylic acids such as 2-hydroxyethyl acrylate, 2-hydroxyethyl methacrylate and 2-hydroxypropyl methacrylate; and (18) monomers having a hydroxyl group such as 4-(1-hydroxy-1-methylbutyl)styrene and 4-(1-hydroxy-1-methylhexyl)styrene.

In the toner of the present invention, vinyl polymers or copolymers of the binder resin may have the cross-linked structure wherein they are cross-linked by a cross-linker having 2 or more vinyl groups. Examples of the cross-linkers used in such a case include aromatic divinyl compounds such as divinylbenzene and divinylnaphthalene. Examples of diacrylate compounds connected by an alkyl chain include ethylene glycol diacrylate, 1,3-butylene glycol diacrylate, 1,4-butanediol diacrylate, 1,5-pentanediol diacrylate, 1,6-hexanediol diacrylate, neopentyl glycol diacrylate, or those wherein the acrylate of the above compounds is replaced by methacrylate.

Examples of the diacrylate compounds connected by an alkyl chain including ether bond include diethyleneglycol diacrylate, triethylene glycol diacrylate, tetraethylene glycol diacrylate, polyethylene glycol #400 diacrylate, polyethylene glycol #600 diacrylate, dipropylene glycol diacrylate, or those wherein the acrylate of the above compounds is replaced by methacrylate.

In addition to the above examples, examples also include diacrylate compounds and dimethacrylate compounds connected by a chain comprising an aromatic group and ether bond. Examples of polyester diacrylates include trade name: MANDA (by Nippon Kayaku Co., Ltd.).

Examples of polyfunctional cross-linkers include pentaerythritol triacrylate, trimethylolethane triacrylate, trimethylolpropane triacrylate, tetramethylolmethane tetraacrylate, oligoester acrylate, those wherein the acrylate of the above compounds is replaced by methacrylate, triallyl cyanurate and triallyl trimellitate.

These cross-linkers can be preferably used in an amount of 0.01 to 10 parts by weight to 100 parts by weight of other monomer components, and particularly preferably used in an amount of 0.03 to 5 parts by weight. Among these cross-linked monomers, examples of the preferably used monomers in a resin for toners in terms of fixity and anti-offset property include aromatic divinyl compounds (particularly preferably divinyl benzene) and diacrylate compounds connected by a binding chain which comprises an aromatic group and one ether bond. Among them, it is preferable to select combination of monomers so as to become a styrene copolymer or a styrene-acrylate copolymer.

In the present invention, examples of polymerization initiators used for producing the vinyl polymer or the copolymer include 2,2'-azobisisobutyronitrile, 2,2'-azobis(4-methoxy-2,4-dimethylvaleronitrile), 2,2'-azobis(2,4-dimethylvaleronitrile), 2,2'-azobis(2-methylbutyronitrile), dimethyl-2,2'-azobisisobutyrate, 1,1'-azobis(1-cyclohexanecarbonitrile), 2-(carbamoylazo)-isobutyronitrile, 2,2'-azobis(2,4,4-trimethylpentane), 2-phenylazo-2',4'-dimethyl-4'-methoxyvaleronitrile, 2,2'-azobis (2-methylpropane), ketone peroxides such as methyl ethyl ketone peroxide, acetyl acetone peroxide and cyclohexanone peroxide, 2,2-bis(tert-butyl peroxy)butane, tert-butyl hydroperoxide, cumenehydroperoxide, 1,1,3,3-tetramethyl butyl hydroperoxide, di-tert-butyl peroxide, tert-butyl cumyl peroxide, dicumyl peroxide, α-(tert-butylperoxy)isopropyl benzene, isobutyl peroxide, octanoyl peroxide, decanoyl peroxide, lauroyl peroxide, 3,5,5-trimethyl hexanoyl peroxide, benzoyl peroxide, m-tolyl peroxide, diisopropyl peroxydicarbonate, di-2-ethylhexyl peroxydicarbonate, di-n-propyl peroxydicarbonate, di-2-ethoxyethyl peroxycarbonate, diethoxy isopropyl peroxydicarbonate, bis(3-methyl-3-methoxybutyl)peroxycarbonate, acetyl cyclohexyl sulfonyl peroxide, tert-butyl peroxyacetate, tert-butyl peroxyisobutyrate, tert-butylperoxy-2-ethylhexalate, tert-butyl peroxylaurate, tert-butyloxy benzoate, tert-butylperoxy isopropyl carbonate, di-tert-butyl peroxyisophthalate, tert-butylperoxy allyl carbonate, isoamyl peroxy-2-ethylhexanoate, di-tert-butylperoxy hexahydroterephthalate and tert-butyl peroxyazelate.

When the binder resin is a styrene-acrylate resin, in the molecular weight distribution of tetrahydrofuran (hereinafter referred to as THF) soluble parts of the resin component with the gel permeation chromatography (hereinafter referred to as GPC), a resin having at least one peak in the molecular weight area of 3,000 to 50,000 (number-average molecular weight) and having at least one peak in the molecular weight area of 100,000 or more is preferable in terms of fixity, offset property and preservative quality. As for THF soluble parts, the binder resin is preferable wherein the component having the molecular weight area of 100,000 or less is 50 to 90%. Further, a resin having the main peak in the molecular weight area of 5,000 to 30,000 is more preferable, and a resin having the main peak in the molecular weight area of 5,000 to 20,000 is most preferable.

When the binder resin is a vinyl polymer such as a styrene-acrylate resin, the acid number thereof is preferably 0.1mgKOH/g to 100mgKOH/g, more preferably 0.1mgKOH/g to 70mgKOH/g, and further more preferably 0.1mgKOH/g to 50mgKOH/g.

Examples of monomers which comprise polyester polymers include the followings.

As bivalent alcohols, they include ethylene glycol, propylene glycol, 1,3-butanediol, 1,4-butanediol, 2,3-butanediol, diethylene glycol, triethylene glycol, 1,5-pentanediol, 1,6-hexanediol, neopentyl glycol, 2-ethyl-1,3-hexanediol, bisphenol A hydride and diols obtained by polymerization of bisphenol A and cyclic ethers such as ethylene oxide and propylene oxide.

It is preferable to combine trivalent or more alcohols in order to cross-link polyester resins. Examples of the trivalent or more alcoholds include sorbitol, 1,2,3,6-hexanetetrol, 1,4-sorbitan, pentaerythritol, dipentaerythritol, tripentaerythritol, 1,2,4-butanetriol, 1,2,5-pentatriol, glycerol, 2-methylpropane triol, 2-methyl-1,2,4-butanetriol, trimethylolethane, trimethylolpropane and 1,3,5-trihydroxybenzene.

Examples of the acid components which constitute the polyester polymers include benzene dicarboxylic acids or anhydrides thereof such as a phthalic acid, isophthalic acid and terephthalic acid; alkyl dicarboxylic acids or anhydrides thereof such as a succinic acid, adipic acid, sebacic acid and azelaic acid; unsaturated dibasic acids such as a maleic acid, citraconic acid, itaconic acid, alkenyl succinic acid, fumaric acid and mesaconic acid; and unsaturated dibasic acid anhydrides such as maleic anhydride, citraconic anhydride, itaconic anhydride and alkenyl succinic anhydride. Examples of the polyvalent (trivalent or more) carboxylic acid components include a trimellitic acid, pyromellitic acid, 2,5,7-naphthalene tricarboxylic acid, 1,2,4-naphthalene tricarboxylic acid, 1,2,4-butane tricarboxylic acid, 1,2,5-hexane tricarboxylic acid, 1,3-dicarboxy-2-methyl-2-methylene carboxypropane, tetra(methylene carboxy)methane, 1,2,7,8-octane tetracarboxylic acid, empol trimeric acids, anhydrides thereof, and partially lower alkyl esters.

When the binder resin is a polyester resin, in the molecular weight distribution of THF soluble parts of the resin component, a resin having at least one peak in the molecular weight area of 3,000 to 50,000 is preferable in terms of fixity and anti-offset property of the toner. As for THF soluble parts, the binder resin is preferable wherein the component having the molecular weight area of 100,000 or less is 60 to 100%. Further, a resin having at least one peak in the molecular weight area of 5,000 to 20,000 is more preferable.

In the present invention, the molecular weight distribution of the binder resin is determined by GPC using THF as a solvent.

When the binder resin is a polyester resin, the acid number thereof is preferably 0.1mgKOH/g to 100mgKOH/g, more preferably 0.1mgKOH/g to 70mgKOH/g, and further more preferably 0.1mgKOH/g to 50mgKOH/g.

Further, the hydroxyl value is preferably 30mgKOH/g or less, and more preferably 10mgKOH/g to 25mgKOH/g.

It is possible to combine two or more kinds of a noncrystalline polyester resin(s) and a crystalline polyester resin(s) and use them in the present invention. In such a case, materials are preferably selected in consideration of compatibility of each material.

As a noncrystalline polyester resin, a polycarboxylic acid component, more preferably a compound synthesized from an aromatic polycarboxylic acid and a polyalcohol component is used.

As a crystalline polyester resin, a dicarboxylic acid component, more preferably a compound synthesized from an aliphatic dicarboxylic acid and a dialcohol component is used.

As the binder resin which can be used in the toner of the present invention, it is possible to use, in the vinyl polymer component and/or the polyester resin component, a resin containing a monomer which can react with both resin components. Among the monomers which constitute the polyester resin component, examples of those which can react with the vinyl polymers include unsaturated dicarboxylic acids or anhydrides thereof such as a phthalic acid, maleic acid, citraconic acid and itaconic acid. Examples of the monomers which constitute the vinyl polymer component include those comprising a carboxyl group or a hydroxyl group and esters of acrylic acids or methacrylic acids.

When combining the polyester polymers, vinyl polymers and other binder resins, it is preferable to contain 60 mass% or more of the resin wherein the acid number of the total binder resin is 0.1 to 50mgKOH/g.

In the present invention, the acid number of the binder resin component of a toner composition is determined by the following method. The basic operation is based on JIS K-0070.
(1) A sample is used after removing additives other than the binder resin (a polymer component), or the acid number and the content of each components other than the binder resin and the cross-linked binder resin are determined in advance. 0.5 to 2.0g of the crushed sample was precisely weighed. The weight of the polymer component is defined as Wg. For example, when the acid number of the binder resin is determined from a toner, the acid number and the content of each of a coloring agent, a magnetic material or the like are separately determined. Then, the acid number of the binder resin is calculated.
(2) The sample is poured in a 300mL beaker. Then, 150mL of a mixed solution of toluene/ethanol (volume ratio = 4/1) is added thereto and dissolved.
(3) The mixed solution is tiltrated using 0.1mol/L of a KOH ethanol solution with a potentiometric tiltrator.
(4) The usage of the KOH solution in (3) is defined as S(mL). At the same time, the blank is determined and the usage of the KOH solution at that time is defined as B(mL). Then, the acid number is calculated using the following formula (1). Meanwhile, f is a factor of the KOH concentration. $Acid number \left(mgKOH/g\right) = \left[\left(S-B\right)\times f\times 5.61\right] / W$

As for the binder resin of a toner and compositions containing the binder resin, the glass transition temperature (Tg) thereof is preferably 35 to 80°C and particularly preferably 40 to 75°C, in terms of the preservative quality of a toner. When Tg is lower than 35°C, a toner easily deteriorates in high temperature atmosphere and offset easily occurs upon fixing. When Tg is higher than 80°C, fixity tends to lower.

In the polymerized toner of the present invention, the binder resin of which softening point is 80 to 140°C is preferably used. When the softening point of the binder resin is lower than 80°C, the toner after fixing and in storage and the image stability thereof sometimes deteriorate. On the other hand, when the softening point of the binder resin is higher than 140°C, the low temperature fixity of the toner sometimes deteriorates.

Examples of the magnetic materials which can be used in the present invention are followings: (1) magnetic iron oxides such as magnetite, maghemite and ferrite, and iron oxides containing other metallic oxides; (2) metals such as iron, cobalt and nickel, or alloyed metals of said metals and the metals such as aluminum, cobalt, copper, lead, magnesium, tin, zinc, antimony, beryllium, bismuth, cadmium, calcium, manganese, selenium, titanium, tungsten and vanadium; and (3) mixtures thereof.

Specific examples of the magnetic materials are Fe₃O₄, γ -Fe₂O₃, ZnFe₂O₄, Y₃Fe₅O₁₂, CdFe₂O₄, Gd₃Fe₅O₁₂, CuFe₂O₄, PbFe₁₂O, NiFe₂O₄, NdFe₂O, BaFe₁₂O₁₉, MgFe₂O₄, MnFe₂O₄, LaFeO₃, iron powder, cobalt powder and nickel powder. The above mentioned magnetic materials are used by itself or by combination of two kinds or more of them. A particularly preferable magnetic material is fine powders of ferrosoferric oxide or γ -iron sesquioxide.

In addition, magnetic iron oxides such as magnetite, maghemite, ferrite, etc containing dissimilar elements or the mixtures thereof are also usable. Examples of the dissimilar elements include lithium, beryllium, boron, magnesium, aluminum, silicon, phosphorus, germanium, zirconium, tin, sulfur, calcium, scandium, titanium, vanadium, chromium, manganese, cobalt, nickel, copper, zinc and gallium. The preferable dissimilar elements are selected from the group consisting of magnesium, aluminum, silicon, phosphorus and zirconium. The dissimilar elements may be incorporated in the crystal lattice of iron oxides or in the iron oxides themselves as oxides, or they may exist on the surface of iron oxides as oxides or hydroxides. It is preferable that the dissimilar elements are contained as oxides.

The above dissimilar elements can be incorporated in the particles by the steps comprising of mixing salts of each dissimilar elements upon producing a magnetic material, and then adjusting pH thereof. Further, the dissimilar elements can be precipitated on the surface of the particles by the steps comprising of adjusting pH thereof after the production of the magnetic particles, or adding salts of each dissimilar elements and adjusting pH thereof.

The usage of the magnetic materials is 10 to 200 parts by weight and preferably 20 to 150 parts by weight to 100 parts by weight of the binder resin. The number average particle diameter of these magnetic materials is preferably 0.1 to 2µm and more preferably 0.1 to 0.5µm. The number average particle diameter can be determined by taking a magnified photograph of the particles with a transmission electron microscope and then measuring it with a digitizer or the like.

As for the magnetic characteristics of the magnetic materials, it is preferable that, when 10K Oersted is applied, the magnetic characteristics are coercivity of 20 to 150 Oersted, saturated magnetization of 50 to 200emu/g, and remanent magnetization of 2 to 20emu/g.

The magnetic materials can also be used as coloring agents. Examples of the coloring agents usable in the present invention include, in the case of a black toner, black or blue dye compounds or pigments. Examples of the black or blue pigments include carbon black, aniline black, acetylene black, phthalocyanine blue and indanthrene blue. Examples of the black or blue dye compounds include azo dye compounds, anthraquinone dye compounds, xanthene dye compounds and methine dye compounds.

When using coloring agents for color toners, examples of the coloring agents are the followings. Examples of magenta coloring agents include condensed azo compounds, diketopyrrolopyrrole compounds, anthraquinone compounds, quinacridone compounds, basic dye compounds, lake dye compounds, naphthol dye compounds, benzimidazolone compounds, thioindigo compounds and perylene compounds. More specifically, examples of the pigmentary magenta coloring agents include C.I. pigment red 1, 2, 3, 4, 5, 6, 7, 8, 9, 10, 11, 12, 13, 14, 15, 16, 17, 18, 19, 21, 22, 23, 30, 31, 32, 37, 38, 39, 40, 41, 48, 49, 50, 51, 52, 53, 54, 55, 57, 58, 60, 63, 64, 68, 81, 83, 87, 88, 89, 90, 112, 114, 122, 123, 163, 202, 206, 207, 209; C.I. pigment violet 19; C.I. vat red 1, 2, 10, 13, 15, 23, 29, 35.

Though it is acceptable to use the above pigment by itself, it is preferable in terms of the image quality of full-color images to combine the dye compound and the pigment so as to improve the color definition.

Examples of dye magenta coloring agents include oil soluble dye compounds such as C.I. solvent red 1, 3, 8, 23, 24, 25, 27, 30, 49, 81, 82, 83, 84, 100, 109, 121; C.I. disperse red 9; C.I. solvent violet 8, 13, 14, 21, 27; C.I. disperse violet 1; and basic dye compounds such as C.I. basic red 1, 2, 9, 12, 13, 14, 15, 17, 18, 22, 23, 24, 27, 29, 32, 34, 35, 36, 37, 38, 39, 40; and C.I. basic violet 1, 3, 7, 10, 14, 15, 21, 25, 26, 27, 28.

It is possible to use, as cyan coloring agents, copper phthalocyanine compounds and derivatives thereof, anthraquinone, and basic dye lake compounds. More specifically, examples of pigmentary cyan coloring agents include C.I. pigment blue 2, 3, 15, 16, 17; C.I. vat blue 6; C.I. acid blue 45; and copper phthalocyanine pigments wherein 1 to 5 phthalimidemethyl group(s) is substituted to a phthalocyanine skeleton.

Examples of yellow coloring agents include condensed azo compounds, isoindolinone compounds, anthraquinone compounds, azo metal complexes, methine compounds and allylamide compounds. More specifically, examples of yellow pigments include C.I. pigment yellow 1, 2, 3, 4, 5, 6, 7, 10, 11, 12, 13, 14, 15, 16, 17, 23, 65, 73, 83; and C.I. vat yellow 1, 3, 20.

Examples of orange pigments include chrome reddish yellow, molybdenum orange, permanent orange GTR, pyrazolone orange, vulcan orange, benzidine orange G, indanthrene brilliant orange RK, and indanthrene brilliant orangeGK. Examples of violet pigments include manganese violet, fast violet B, and methyl violet lake. Examples of green pigments include chrome oxides, chrome green, pigment green, malachite green lake, and final yellow green G. Examples of white pigments include Chinese white, titanium oxides, antimony white, and zinc sulfide.

The usage of the above coloring agents is preferably 0.1 to 20 parts by weight to 100 parts by weight of the binder resin.

The toner of the present invention may be mixed with a carrier to be used as a two component developer. As for the carriers used in the present invention, it is possible to use both usual carriers such as ferrite and magnetite and resin coated carriers.

The resin coated carrier comprises carrier core particles and a coating material which is a resin coating the surface of the carrier core particles. Preferable examples of the resins used as the coating material include styrene-acrylate resins such as styrene-acrylic acid ester copolymers and styrene-methacrylic acid ester copolymers; acrylate resins such as acrylic acid ester copolymers and methacrylic acid ester copolymers; fluorine-containing resins such as polytetrafluoroethylene, monochlorotrifluoroethylene polymers and polyvinylidene-fluoride; silicone resins; polyester resins; polyamide resins; polyvinyl butyral; and aminoacrylate resins. In addition to them, examples include resins which can be used as a coating material of the carrier such as iomonomer resins and polyphenylene sulfide resins. These resins are used by itself or by combination of two or more kinds of them.

Besides, a binder carrier core wherein magnetic powders are dispersed in a resin is also usable.

As for the method of coating the surface of a carrier core with at least a resin coating agent in a resin coated carrier, it is possible to apply the method comprising the steps of dissolving or suspending a resin in a solvent, and making the solvent adhere on the carrier core to be coated; or the method of simply mixing a resin in a powdery condition. The ratio of the resin coating material to the resin coated carrier can be properly determined, and it is preferably 0.01 to 5 mass% to the resin coated carrier and more preferably 0.1 to 1 mass%.

The usage examples of a coating agent comprising a mixture of two or more kinds of compounds for coating a magnetic material include: (1) a coating agent treated with 12 parts by weight of a mixture of dimethyldichlorosilane and dimethyl silicon oil (mass ratio = 1:5) to 100 parts by weight of fine powders of a titanium oxide; and (2) a coating agent treated with 20 parts by weight of a mixture of dimethyldichlorosilane and dimethyl silicon oil (mass ratio = 1:5) to 100 parts by weight of fine powders of silica.

Among the above resins, a styrene-methyl methacrylate copolymer, a mixture of a fluorine-containing resin and a styrene copolymer, or a silicone resin is preferably used. Particularly, a silicone resin is preferable.

Examples of the mixture of a fluorine-containing resin and a styrene copolymer include a mixture of polyvinylidene-fluoride and a styrene-methyl methacrylate copolymer, a mixture of polytetrafluoroethylene and a styrene-methyl methacrylate copolymer, and a mixture of a vinylidene fluoride-tetrafluoroethylene copolymer (copolymer mass ratio = 10:90-90:10), a styrene-acrylic acid-2-ethylhexyl copolymer (copolymer mass ratio = 10:90-90:10) and a styrene-acrylic acid-2-ethylhexyl-methyl methacrylate copolymer (copolymer mass ratio = 20-60:5-30:10:50).

Examples of the silicone resin include modified silicone resins which are produced by the reaction of a silicone resin with a nitrogen-containing silicone resin(s) and a nitrogen-containing silane coupling agent(s).

As for magnetic materials of a carrier core, it is possible to use oxides such as ferrite, iron excess ferrite, magnetite and γ-iron oxide; metals such as iron, cobalt and nickel; or alloyed metals of said metals. Examples of elements contained in these magnetic materials include iron, cobalt, nickel, aluminum, copper, lead, magnesium, tin, zinc, antimony, beryllium, bismuth, calcium, manganese, selenium, titanium, tungsten and vanadium. The preferable ones are copper-zinc-iron ferrite comprising copper, zinc and iron as main components, and manganese-magnesium-iron ferrite comprising manganese, magnesium and iron as main components.

The resistance value of a carrier is preferably adjusted to 10⁶ to 10¹⁰ Ω /cm by adjusting concavity and convexity of the surface of the carrier and the amount of the resin to be coated. As for the particle diameter of the carrier, though the particle diameter of 4 to 200µm can be used, 10 to 150µ m is preferable and 20 to 100µm is more preferable. Particularly, a resin coated carrier preferably has 50% particle diameter of 20 to 70µm.

In a two component developer, it is preferable to use the toner of the present invention in an amount of 1 to 200 parts by weight to 100 parts by weight of the carrier. It is more preferable to use the toner in an amount of 2 to 50 parts by weight to 100 parts by weight of the carrier.

The toner of the present invention may further contain a wax. Examples of the wax used in the present invention include the followings: aliphatic hydrocarbon waxes such as low-molecular-weight polyethylene, low-molecular-weight polypropylene, polyolefin wax, microcrystalline wax, paraffin wax and Sasol wax; oxides of aliphatic hydrocarbon waxes such as oxidized polyethylene wax; block copolymers thereof; botanical waxes such as candelilla wax, carnauba wax, Japan wax and jojoba wax; animal waxes such as bees wax, lanolin and whale wax; mineral waxes such as ozokerite, ceresin and petrolatum; waxes comprising fatty acid esters as a main component, such as wax of montanic acid esters and castor wax; and partially or wholly deoxidized fatty acid esters such as deoxidized carnauba wax.

Further examples of the wax include saturated straight fatty acids such as a palmitic acid, stearic acid, montanic acid and straight alkyl carboxylic acids further comprising a straight alkyl group; unsaturated fatty acids such as a brassidic acid, eleostearic acid and parinaric acid; saturated alcohols such as stearyl alcohol, eicosyl alcohol, behenyl alcohol, carnaubil alcohol, ceryl alcohol, mesilyl alcohol and long-chain alkyl alcohol; polyalcohols such as sorbitol; fatty acid amides such as linoleic acid amide, olefinic acid amide and lauric acid amide; saturated fatty acid bisamides such as methylene bis-capric acid amide, ethylene bis-lauric acid amide and hexamethylene bis-stearic acid amide; unsaturated fatty acid amides such as ethylene bisoleic acid amide, hexamethylene bisoleic acid amide, N,N'-dioleyl adipic acid amide and N,N'-dioleyl sebacic acid amide; aromatic bisamides such as m-xylene bis-stearic acid amide and N,N'-distearyl isophthalic acid amide; metallic salts of fatty acids such as calcium stearate, calcium laurate, zinc stearate and magnesium stearate; waxes wherein an aliphatic hydrocarbon wax is grafted by using a vinyl monomer such as styrene and acrylate; partially esterified compounds of polyalcohol and a fatty acid such as behenic acid monoglyceride; and methylester compounds having a hydroxyl group which are obtained by hydrogenating a vegetable oil.

Examples of the preferably used wax include polyolefin obtained by radical-polymerizing olefin under high pressure; polyolefin obtained by purifying a low-molecular-weight by-product obtained in the polymerization of high-molecular-weight polyolefin; polyolefin polymerized under low pressure by using a catalyst such as Ziegler catalyst and metallocene catalyst; polyolefin polymerized by using radiation, electromagnetic wave or light; low-molecular-weight polyolefin obtained by thermally decomposing high-molecular-weight polyolefin; paraffin wax, microcrystalline wax and Fischer-Tropsch wax; synthetic hydrocarbon waxes synthesized by Synthol process, Hydrocol process, Arge process, or the like; synthetic waxes having a compound of one carbon atom as a monomer; hydrocarbon waxes having a functional group such as a hydroxyl group and a carboxyl group; a mixture of a hydrocarbon wax and a hydrocarbon wax having a functional group; and waxes wherein the above waxes are grafted by a vinyl monomer such as styrene, ester maleate, acrylate, methacrylate and maleic anhydride.

Further, it is preferable to use waxes of which molecular weight distribution is sharpened by treating them with Press sweating process (method), solvents, recrystallization method, vacuum distillation method, supercritical gas extraction method or solution crystallization method; or waxes from which low-molecular-weight solid fatty acids, low-molecular-weight solid alcohols, low-molecular-weight solid compounds or other impurities are removed.

The wax used in the present invention preferably has the melting point of 50 to 140°C and more preferably 70 to 120°C in order to balance fixity and anti-offset property When the melting point is lower than 50°C, the blocking resistance decreases. When the melting point is higher than 140°C, the anti-offset effect is less likely to occur.

Further, combination of two or more different kinds of waxes can develop both the plasticizing action and the mold-releasing action at the same time, each of which is the action of waxes.

Examples of waxes having the plasticizing action are waxes having a low melting point, those having a branched molecular structure, and those having a polar group in the structure. Examples of waxes having the mold-releasing action are waxes having a high melting point, those having a straight molecular structure, and those having nonpolar molecules which do not have any functional group. As usage examples, there are the combination of two or more kinds of waxes between which the difference of the melting points is 10 to 100°C; and the combination of polyolefin and grafted polyolefin.

When selecting two kinds of waxes, in the case of the waxes having the similar structure, the wax which relatively has lower melting point exerts the plasticizing action, and the wax which relatively has higher meting point exerts the mold-releasing action. At that time, when the difference of each melting points is 10 to 100°C, the functional separation is effectively exerted. When the difference is less than 10°C, the effect of the functional separation is less likely to occur, and when it is more than 100°C, the accentuation of each functions by the interaction is less likely to occur. In such a case, when at least one of the waxes preferably has the melting point of 70 to 120°C and more preferably 70 to 100°C, the waxes tend to easily exert the effect of the functional separation.

Besides, the wax which relatively has a branched molecular structure, has a polar group or is modified by a component different from the main component exerts the plasticizing action. The wax which relatively has a straight molecular structure, has nonpolar molecules which do not have any functional group or is unmodified and straight exerts the mold-releasing action. Examples of the preferable combination thereof include a combination of polyethylene homopolymer or copolymer having ethylene as the main component and polyolefin homopolymer or copolymer having olefin other than ethylene as the main component; a combination of polyolefin and grafted polyolefin; a combination of a hydrocarbon wax and an alcohol wax, a fatty acid wax or an ester wax; a combination of Fischer-Tropsch wax or a polyolefin wax and a paraffin wax or a microcrystalline wax; a combination of Fischer-Tropsch wax and a polyolefin wax; a combination of a paraffin wax and a microcrystalline wax; and a combination of a hydrocarbon wax and a carnauba wax, a candelilla wax, a rice bran wax or a montan wax.

In each case, in the endothermic peak observed in the DSC measurement of the toner, it is preferable that the peak-top temperature of the maximum peak is within 70 to 110°C. It is more preferable that the maximum peak is within 70 to 110°C. This makes it easier to balance the preservative quality and the fixity of the toner.

In the toner of the present invention, it is effective to use these waxes in a total content of preferably 0.2 to 20 parts by weight and more preferably 0.5 to 10 parts by weight to 100 parts by weight of the binder resin.

In the present invention, the melting point of a wax is defined as the peak-top temperature of the maximum peak in the endothermic peak of the wax observed in DSC.

In the present invention, it is preferable to conduct the DSC measurement of the wax or the toner with a high-precision intraheater power-compensation type differential scanning calorimeter. The measurement method is based on ASTM D3418-82. The DSC curve used in the present invention is the curve measured when a sample is heated at temperature velocity of 10°C/min. after heating and cooling the sample once and taking a record in advance.

A flow improver may be added to the toner of the present invention. A flow improver improves flowability of the toner (makes it easier to flow) by being added to the surface of the toner. Examples thereof include fluorine resin powders such as carbon black, fine powders of vinylidene fluoride and fine powders of polytetrafluoroethylene; fine powders of silica such as wet processed silica and dry processed silica; fine powders of unoxidized titanium; fine powders of alumina; and treated silica, treated titanium oxide and treated alumina wherein each of the above fine powders is surface-treated with a silane coupling agent, titanium coupling agent or silicone oil. Among them, fine powders of silica, fine powders of unoxidized titanium and fine powders of alumina are preferable, and the treated silica wherein each of said fine powders is surface-treated with a silane coupling agent or silicone oil is further more preferable. The particle diameter of the flow improver is preferably 0.001 to 2µm as the average primary particle diameter and particularly preferably 0.002 to 0.2µm.

The preferable fine powders of silica are fine powders produced by oxidizing the gas phase of silicon halides, and referred to as dry processed silica or fumed silica.

Examples of the marketed silica fine powders produced by oxidizing the gas phase of silicon halides include the following trade names: AEROSIL-130, -300, -380, -TT600, -MOX170, -MOX80 and -COK84 (all produced by Nippon Aerosil Co., Ltd.); Ca-O-SiL-M-5, -MS-7, -MS-75, -HS-5 and -EH-5 (all produced by CABOT K.K.); Wacker HDK-N20 V15, -N20E, -T30 and -T40 (all produced by Wacker -Chemie GmbH); D-C FineSilica (produced by Dow Corning Toray Co., Ltd.); and Franso 1 (produced by Fransil K.K.).

In addition, treated silica fine powders wherein the silica fine powders produced by oxidizing the gas phase of silicon halides are hydrophobized is more preferable. Among the treated silica fine powders, those each of which is treated so that the hydrophobizing degree thereof measured in methanol titration test preferably indicates 30 to 80% are particularly preferable. Hydrophobizing is given by chemically or physically treating silica fine powders with an organic silicon compound(s) which reacts with silica fine powders or physically adsorbs to them. The preferable method is that comprising the step of treating silica fine powders produced by oxidizing the gas phase of silicon halides with an organic silicon compound(s).

Examples of the organic silicon compound include hydroxypropyl trimethoxysilane, phenyltrimethoxysilane, n-hexadecyltrimethoxysilane, n-octadecyltrimethoxysilane, vinylmethoxysilane, vinyltriethoxysilane, vinyltriacetoxysilane, dimethylvinylchlorosilane, divinylchlorosilane, γ -methacryloxypropyltrimethoxysilane, hexamethyldisilane, trimethylsilane, trimethylchlorosilane, dimethyldichlorosilane, methyltrichlorosilane, allyldimethylchlorosilane, allylphenyldichlorosilane, benzyldimethylchlorosilane, bromomethyldimethylchlorosilane, α -chloroethyltrichlorosilane, β -chloroethyltrichlorosilane, chloromethyldimethylchlorosilane, triorganosilyl mercaptan, trimethylsilyl mercaptan, triorganosilyl acrylate, vinyldimethylacetoxysilane, dimethylethoxysilane, trimethylethoxysilane, trimethylmethoxysilane, methyltriethoxysilane, isobutyltrimethoxysilane, dimethyldimethoxysilane, diphenyldiethoxysilane, hexamethyldisiloxane, 1,3-divinyltetramethyldisiloxane, 1,3-diphenyltetramethyldisiloxane and dimethylpolysiloxane which has 2 to 12 siloxane units per one molecule and contains 0 to 1 hydroxyl group attached to Si in each unit located on ends. Further, examples include silicone oils such as dimethylsilicone oil. Each of the above compounds is used by itself or by a mixture of two or more kinds of them.

The number average particle diameter of the flow improver is preferably 5 to 100nm and more preferably 5 to 50nm. The specific surface area thereof by the nitrogen adsorption measured by BET method is preferably 30m²/g or more and more preferably 60 to 400m²/g. The specific surface area of the surface-treated fine powders is preferably 20m²/g or more and particularly preferably 40 to 300m²/g. The preferable applied amount of these fine powders is 0.03 to 8 parts by weight to 100 parts by weight of toner particles.

To the toner of the present invention, it is possible to add other additives such as various metallic soaps, fluorine surfactants and dioctyl phthalate; conductivity giving agents such as tin oxide, zinc oxide, carbon black and antimony oxide; or inorganic fine powders of titanium oxide, aluminum oxide and alumina, if necessary, in order to protect a photoreceptor and a carrier, improve cleaning property, control heat property, electric property, and physical property, control resistance, control softening point and improve the fixation ratio. These inorganic fine powders may be hydrophobized, if necessary. Further, it is possible to use, as an image development improver, a small amount of lubricants such as polytetrafluoroethylene, zinc stearate and polyvinylidene-fluoride; abrasives such as cesium oxide, silicon carbide and strontium titanate; anticaking agents; or white microparticles and black microparticles each of which have the opposite polarity of the toner particles.

It is also preferable to treat the above additives with silicone varnish, various modified silicone varnishes, silicone oil, various modified silicone oils, silane coupling agents, silane coupling agents having a functional group(s), treatment agents such as other organic silicon compounds or various other treatment agents, in order to control the charge amount.

In the present invention, the charge control agent can be sufficiently mixed by stirring with the above additive(s) and the toner by a mixer such as Henschel mixer, a ball mill, Nauta mixer, a V-type mixer, a W-type mixer and a supermixer; and said mixture be uniformly externally added to the surface of the toner particles to obtain the subject toner for static charge development.

Since the toner of the present invention is thermally stable and not changed by heat in the process of electrophotography, it is possible to maintain stable charging characteristics. In addition, since the toner uniformly disperses in any binder resin, the charging distribution of a fresh toner is fairly uniform. Accordingly, as for the toner of the present invention, changes are hardly seen in both the saturated frictional charge amount and the charging distribution of the untransferable toner and the collected toner (a discarded toner) thereof as compared with those of the fresh toner. When reusing the discarded toner collected from the toner for static charge image development of the present invention, the gap between the fresh toner and the discarded toner can be further reduced by selecting a polyester resin containing aliphatic diol as the binder resin, or by producing the toner in accordance with the method comprising the steps of selecting a metal-bridged styrene-acrylate copolymer as the binder resin and adding large quantities of polyolefin thereto.

As for the method of producing the toner of the present invention, the toner can be produced by the known production method. For example, the preferable production method is the method (crushing method) comprising the steps of sufficiently mixing the above mentioned toner constituent materials such as a binder resin, a charge control agent and a coloring agent by a mixer such as a ball mill; then, sufficiently kneading the mixture by a heat kneading machine such as a heat roll kneader; solidifying by cooling, crushing and classifying the mixture to obtain a toner.

The toner can also be produced by dissolving the above mixture in a solvent, atomizing, drying and classifying it. Further, the toner can also be produced by the polymerization method, which comprises the steps of mixing specific materials to a monomer constituting the binder resin to prepare an emulsion or a suspension, and polymerizing the solution. As for a microcapsule toner comprising a core material and a shell material, such toner can be produced by the method comprising the step of making specific materials contain in a core material or a shell material, or both of them. Further, if necessary, the toner of the present invention can be produced by sufficiently mixing a needed additive(s) and toner particles by a mixer such as Henschel mixer.

The method of producing the toner of the present invention by the above crushing method is further illustrated as follows. First, a binder resin, a coloring agent, a charge control agent and other necessary additives are uniformly mixed. They can be mixed with a known mixer such as Henschel mixer, a supermixer and a ball mill. The obtained mixture is heat-molten and kneaded with a hermetically sealed kneader or a single or double screw extruder. After cooling down the kneaded mixture, it is coarsely crushed with a crusher or a hammer mill, and then finely milled with a pulverizer such as a jet mill and a high-speed rotor whirling mill. Then, the obtained powders are classified to a specific particle size with a wind force classifier such as Elbow-jet of an inertial classification system utilizing the Coanda effect, Microplex of a cyclone (centrifugal) classification system or a DS separator. When further adding an external additive(s) to the surface of the toner, the toner and the external additive(s) are stirred and mixed with a high-speed mixer such as Henschel mixer and a supermixer.

The toner of the present invention can also be produced by the suspension polymerization method or the emulsion polymerization method. The suspension polymerization method comprises the following steps. A polymerizable monomer, a coloring agent, a polymerization initiator, a charge control agent and, if necessary, a cross-linker, a dispersion stabilizer and other additives are uniformly dissolved or dispersed to prepare a monomer composition. The monomer composition is dispersed in the continuous phase containing the dispersion stabilizer and said composition such as the aqueous phase with a suitable mixer or disperser such as a homomixer, a homogenizer, an atomizer, a microfluidizer, a one-fluid nozzle, a gas-liquid fluid nozzle and an electric emulsifying machine. Preferably, the stirring speed, temperature and time are controlled so that droplets of the polymerizable monomer composition have the desired toner particle size, and granulation is conducted. At the same time, the polymerization reaction is conducted at 40 to 90°C to be able to obtain toner particles having the desired particle diameter. The obtained toner particles are washed, filtered out and dried. As for the external addition after producing the toner particles, the above mentioned method can be used.

When producing the toner by the emulsion polymerization method, though the toner particles thereof are more uniform than those obtained by the suspension polymerization method, the average particle diameter thereof is 0.1 to 1.0µm and extremely small. Therefore, in some cases, a toner can be produced by the seed polymerization in which an emulsified particle becomes a core and a polymerizable monomer is added thereto afterward to grow the particle, or by the method comprising the steps of unifying and fusing emulsified particles to a suitable average particle diameter.

According to the production of the toner by these polymerization methods, since there is no crushing process, there is no need to give brittleness to toner particles. Thus, it is possible to use large amounts of substances having a low softening point, of which use was difficult in prior crushing methods, and that makes it possible to widen choices of materials. Further, since a mold-releasing agent or a coloring agent each of which is a hydrophobizing material is not easily exposed on the surface of the toner particles, it is possible to decrease contamination in a toner support member, a photoreceptor, a transferring roller, a fixing machine or the like.

The production of the toner of the present invention by the polymerization method can further improve properties such as image reproducibility, transferability and color reproducibility Further, a toner having a sharp particle size distribution can be comparatively easily obtained by minimizing the particle diameter of the toner in order to apply to tiny dots.

As for the polymerizable monomer used in producing the toner of the present invention by the polymerization method, a vinyl polymerizable monomer of which radical polymerization is possible is used. As the vinyl polymerizable monomer, a monofunctional polymerizable monomer or a polyfunctional polymerizable monomer can be used.

Examples of thy monofunctional polymerizable monomer include styrene polymerizable monomers such as styrene, α-methylstyrene, β -methylstyrene, o-methylstyrene, m-methylstyrene, p-methylstyrene, 2,4-dimethylstyrene, p-n-butylstyrene, p-tert-butylstyrene, p-n-hexylstyrene and p-phenylstyrene; acrylate polymerizable monomers such as methyl acrylate, ethyl acrylate, n-propyl acrylate, isopropyl acrylate, n-butyl acrylate, isobutyl acrylate, tert-butyl acrylate, n-amyl acrylate, n-hexyl acrylate, 2-ethylhexyl acrylate, n-octyl acrylate, benzyl acrylate, dimethylphosphate methyl acrylate, dibutylphosphate ethyl acrylate and 2-benzoyloxy ethyl acrylate; methacrylate polymerizable monomers such as methyl methacrylate, ethyl methacrylate, n-propyl methacrylate, isopropyl methacrylate, n-butyl methacrylate, isobutyl methacrylate, tert-butyl methacrylate, n-amyl methacrylate, n-hexyl methacrylate, 2-ethylhexyl methacrylate, n-octyl methacrylate, diethylphosphate methacrylate and dibutylphosphate ethyl methacrylate; unsaturated aliphatic monocarboxylic acid esters; vinyl esters such as vinyl acetate, vinyl propionate and vinyl benzoate; vinyl ethers such as vinyl methyl ether and vinyl isobutyl ether; and vinyl ketones such as methyl vinyl ketone, hexyl vinyl ketone and isopropyl vinyl ketone.

As a polymerization initiator used when producing the toner of the present invention by the polymerization method, known substances such as organic peroxides can be used. Examples of the water-soluble initiator include ammonium persulfate, potassium persulfate, 2,2'-azobis(N,N'-dimethylene isobutyroamidine) hydrochloride, 2,2'-azobis(2-aminodipropane) hydrochloride, azobis(isobutylamidine) hydrochloride, 2,2'-azobisisobutyronitrile sodium sulfonate, ferrous sulfate and hydrogen peroxide.

The additive amount of a polymerization initiator is preferably 0.5 to 20 parts by weight to 100 parts by weight of a polymerizable monomer. The polymerization initiator may be used by itself or by combination thereof. Examples of the dispersant used in the production of a polymerized toner include inorganic oxides such as tricalcium phosphate, magnesium phosphate, aluminum phosphate, zinc phosphate, calcium carbonate, magnesium carbonate, aluminum hydroxide, calcium metasilicate, calcium sulfate, barium sulfate, bentonite, silica and alumina. As for organic compounds, for example, polyvinyl alcohol, gelatin, methylcellulose, methylhydroxypropylcellulose, ethyl cellulose, sodium salt of carboxymethylcellulose, starch, or the like is used. These dispersants are preferably used in an amount of 0.2 to 2.0 parts by weight to 100 parts by weight of a polymerizable monomer.

Though the marketed dispersants may be used as they are, in order to obtain fine disperse particles having a uniform particle size, the above inorganic compounds can also be produced by high-speed stirring in a disperse medium.

As for the toner obtained by the polymerization method, the concavity and convexity of the toner particles tend to be smaller than those of the toner obtained by the crushing method in which special treatment is not conducted. Since such toner particles are amorphous, the contact area between an electrostatic latent image support member and the toner increases, and it makes the toner adhesion stronger. As a result, the contamination in the machine is decreased and it becomes easier to obtain higher image density and higher quality images.

As for the toner produced by the crushing method, the concavity and convexity of the toner surface can be decreased by the methods such as the hot-water bath method which comprises the steps of dispersing toner particles in water and heating the solution; heat treatment method comprising the step of making toner particles pass through thermal current; and the mechanical impact method comprising the step of treating the particles by giving the mechanical energy Examples of the effective equipments for decreasing the concavity and convexity include a Mechanofusion system (produced by Hosokawa Micron Corp.) applying the dry mechanochemical treatment; an I-type jet mill; a hybridizer (produced by Nara Machinery Co., Ltd.) which is a mixing equipment with a rotor and a liner; and Henschel mixer which is a mixer having high-speed blades.

As one of the values which show the degree of the concavity and convexity of the toner particles, an average circularity degree can be used. The average circularity degree (C) indicates the value which is calculated as follows. First, a circularity degree (Ci) is calculated by the following formula (2). Then, the sum of the circularity degrees of all measured particles is divided by the number of all measured particles (m) as mentioned in the following formula (3). $Circularity degree \left(Ci\right) = \frac{Boundary length of the circle having the same projected area as that of a particle}{Boundary length of the projected image of a particle}$ $Average circularity degree C = {\sum }_{i = 1}^{m} C i / m$

The above circularity degree (Ci) is measured using a flow particle image analyzer such as FPIA-1000 produced by TOA Medical Electronics Co., Ltd. As for the measurement method, first, about 5mg of a toner is dispersed in 10mL of water in which about O.lmg of a nonionic surfactant is dissolved to prepare a dispersion solution. Ultrasonic wave (20kHz, 50W) is irradiated to the dispersion solution for 5 minutes, and the solution is prepared to become the concentration of 5000 to 20000/µL. Then, the distribution of the circularity degree of a particle having the diameter which is equivalent to the circle of 0.60µm or more and less than 159.21µm is measured with the flow particle image analyzer.

The value of the average circularity degree is preferably 0.955 to 0.995. It is further preferable to prepare toner particles so that the value becomes 0.960 to 0.985 since events which cause the increase in the left toner after transferring decrease and another transferring tends not to easily occur.

In the case of the toner of the present invention, in terms of clear images and productivity of the toner, the particle diameter of the crushed toner is preferably 2 to 15µm in the average particle diameter on volumetric basis in the measurement with a laser particle size distribution analyzer such as a micron sizer produced by Seishin Enterprise Co., Ltd, for example. 3 to 12µm thereof is more preferable. When the average particle diameter is beyond 15µm, the resolution or sharpness of images tends to weaken. When the average particle diameter is less than 2µm, though the resolution becomes better, it costs more because of the decrease in the yield rate upon production of a toner. Further, a toner spatters in the machine, or health disorders such as skin penetration tend to occur.

On the other hand, in the case of the polymerized toner, the particle diameter of the toner is preferably 3 to 9µm, more preferably 4 to 8.5µm, and particularly preferably 5 to 8µm. When the average particle diameter thereof on volumetric basis is less than 4µm, the flowability of the toner is decreased and the electrostatic property of each particle tends to lower. Further, since the charging distribution spreads, fogging to the background or toner spilling from the machine tends to easily occur. In addition, when the average particle diameter is less than 4µm, cleaning property sometimes dramatically lowers. When the average particle diameter thereof on volumetric basis is more than 9µm, the resolution of images lowers, and sufficient image quality cannot be obtained. As a result, it is sometimes difficult to satisfy the recent need of obtaining high image quality.

Further, when depicting a cumulative distribution from the small diameter side of each of the volume and the number of particles in the divided particle size range (channel) of the particle size distribution measured by the method mentioned below, the particle diameter of cumulative 16% is defined as volume D16%, that of cumulative 50% is defined as volume D50%, and that of cumulative 84% is defined as volume D84%. At that time, in the polymerized toner of the present invention, a volume average particle size distribution index (GSDv) calculated from (D84%/D16%)1/2 is preferably 1.15 to 1.30 and more preferably 1.15 to 1.25.

As for the particle size distribution of a toner, in the case of the toner of the present invention, it is preferable that the content of particles of 2µm or smaller accounts for 10 to 90% on number basis of the toner, which is measured by a Coulter counter (TA-II, produced by Coulter K.K.), for example. Besides, it is preferable that the content of particles of 12.7µm or larger accounts for 0 to 30% on volumetric basis of the toner.

Further, it is preferable that the uniformity of particle diameters is high (volume average particle diameter/number average particle diameter = 1.00 to 1.30).

In the case of the toner for static charge development of the present invention, it is preferable that the specific surface area of the toner is 1.2 to 5.0m²/g according to the BET specific surface area measurement wherein nitrogen is used as deadsorption gas. It is more preferable that the specific surface area is 1.5 to 3.0m²/g. The measurement of the specific surface area comprises the steps, for example, of desorbing adsorption gas on the surface of the toner at 50°C for 30 minutes with a BET specific surface area measurement device (such as FlowSorbII2300 produced by Shimadzu Corporation); adsorbing nitrogen gas again by rapidly cooling down the toner with liquid nitrogen; and then heating it again up to 50°C. The specific surface area is defined as the value calculated from the amount of desorbed gas at that time.

In the case of the toner of the present invention, the apparent ratio (the powder density) thereof is measured with a powder tester (produced by Hosokawa Micron Corp., for instance), for example. The ratio of a non-magnetic toner is preferably 0.2 to 0.6g/cm³. The ratio of a magnetic toner is preferably 0.2 to 2.0 g/cm³, though it depends on a kind of magnetic powders or the content thereof.

In the case of the toner of the present invention, the absolute specific gravity of a non-magnetic toner is preferably 0.9 to 1.2g/cm³. The absolute specific gravity of a magnetic toner is preferably 0.9 to 4.0g/cm³, though it depends on a kind of magnetic powders or the content thereof. The absolute specific gravity of the toner is calculated as follows. 1.000g of the toner is precisely weighed, poured in a 10mmΦ tableting machine and compressed at a pressure of 200kgf/cm² under vacuum to make tablets. The height of this columnar tablet is measured with a micrometer, and the absolute specific gravity is calculated therefrom.

The flowability of a toner is defined, for example, by a flowing repose angle and a still repose angle measured by a device for measuring the angle of repose (produced by Tsutsui Scientific Instruments Co., Ltd., for example). In the case of the toner for static charge development wherein the charge control agent of the present invention is used, a flowing repose angle is preferably 5 to 45° and a still repose angle is preferably 10 to 50° .

As for the toner of the present invention, the average value of shape factor (SF-1) of the crushed toner is preferably 100 to 400; and the average value of shape factor 2 (SF-2) thereof is preferably 100 to 350.

In the present invention, SF-1 and SF-2 each of which indicates shape factor of the toner were calculated as follows, for example. Toner particles magnified 1000 diameters were taken as a sample so that around 30 particles appear in one visual field by using a light microscope with a CCD camera (such as BH-2 produced by Olympus Corporation). The obtained image was transferred to an image analyzer (such as LUZEX FS produced by Nireco Corporation). The same procedure was repeated until the number of toner particles reaches about 1000 and the shape factor was calculated. Shape factor (SF-1) and shape factor 2 (SF-2) are calculated by the following formulae. $SF - 1 = \left(\left({ML}^{2}\times π\right)/4⁢A\right) \times 100$
wherein, ML is the maximum length of particles; A is a projected area of one particle, $SF - 2 = \left({PM}^{2}/4⁢A⁢π\right) \times 100$
wherein, PM is the peripheral length of particles; A is a projected area of one particle.

SF-1 indicates deformation of a particle. SF-1 becomes closer to 100 when a particle becomes closer to a sphere, and the slenderer a particle is, the larger SF-1 is. SF-2 indicates concavity and convexity of a particle. SF-2 becomes closer to 100 when a particle becomes closer to a sphere, and the more complicated the shape of a particle is, the larger SF-2 is.

The volume resistivity of the toner of the present invention is preferably 1 × 10¹² to 1 × 10¹⁶Ω·cm in the case of a non-magnetic toner. The volume resistivity of a magnetic toner is preferably 1 × 10⁸ to 1 × 10¹⁶ Ω·cm, though it depends on a kind of magnetic powders or the content thereof. Here, the volume resistivity of the toner is defined as follows. Toner particles are compressed to prepare a disk-shaped test piece of 50mm in diameter and 2mm thick. This piece is set to electrodes for solid materials (such as SE-70 produced by Ando Electric Co., Ltd.), and direct voltage 100V is continuously applied to the piece. Then, the value thereof one hour later is measured with a high insulation resistance meter (for example, 4339A produced by Hewlett-Packard Company) and defined as the volume resistivity.

The dielectric tangent of the toner of the present invention is preferably 1.0 × 10⁻³ to 15.0 × 10⁻³ in the case of a non-magnetic toner. The dielectric tangent of a magnetic toner is preferably 2 × 10⁻³ to 30 × 10⁻³, though it depends on a kind of magnetic powders or the content thereof. Here, the dielectric tangent of the toner is defined as follows. Toner particles are compressed to prepare a disk-shaped test piece of 50mm in diameter and 2mm thick. This piece is set to electrodes for solid materials and measured in measurement frequency of 1KHz and peak-to-peak voltage 0.1KV with a LCR meter (for example, 4284A produced by Hewlett-Packard Company). Thus obtained value is defined as the dielectric tangent value (Tan δ).

The Izod impact level of the toner of the present invention is preferably 0.1 to 30kg·cm/cm. Here, the Izod impact level of the toner is measured by the method comprising the steps of fusing toner particles by heat to prepare a plate-like test piece; and measuring the pieces in accordance with JIS K-7110 (Izod impact test of rigid plastic).

The melt index (MI) of the toner of the present invention is preferably 10 to 150g/10min. Here, MI of the toner is measured in accordance with JIS K-7210 (A method), and at that time, the measurement temperature is 125°C and weight is 10kg.

The melting start temperature of the toner of the present invention is preferably 80 to 180°C, and 4mm descent temperature is preferably 90 to 220°C. Here, the melting start temperature of the toner is measured by the following method. Toner particles are compressed to prepare a column-shaped test piece of 10mm in diameter and 20mm thick. This piece is set to a thermofusion property measurement device such as a flowtester (for example, CFT-500C produced by Shimadzu Corporation) and measured in load of 20kgf/cm². Under such condition, the temperature at which the fusion starts and a piston starts to descend is defined as the melting start temperature. Further, in the same measurement, the temperature at which the piston descends 4mm is defined as 4mm descent temperature.

The glass transition temperature (Tg) of the toner of the present invention is preferably 35 to 80°C, and more preferably 40 to 75°C. Here, the glass transition temperature of the toner is measured with a differential scanning calorimetry (hereinafter referred to as DSC) by the method comprising the steps of heating the toner at a constant temperature, rapidly cooling it down, and heating it again. Tg is defined as the value determined from the peak of phase-change which occurs at that time. When Tg of the toner is lower than 35°C, anti-offset property or preservative quality thereof tends to deteriorate. When Tg is higher than 80°C, the fixity level of images tends to deteriorate.

In the endothermic peak observed in the DSC measurement of the toner of the present invention, it is preferable that the peak-top temperature of the maximum peak is within 70 to 120°C.

The melt viscosity of the toner of the present invention is preferably 1000 to 50000 poise and more preferably 1500 to 38000 poise. Here, the melt viscosity of the toner is measured as follows. Toner particles are compressed to prepare a column-shaped test piece of 10mm in diameter and 20mm thick. These pieces are set to a thermofusion property measurement device such as a flowtester (for example, CFT-500C produced by Shimadzu Corporation) and measured in load of 20kgf/cm². Thus measured value is defined as the melt viscosity.

The dissolving residue of a solvent of the toner of the present invention is preferably 0 to 30 mass% as THF insoluble matter, 0 to 40 mass% as ethyl acetate insoluble matter, and 0 to 30 mass% as chloroform insoluble matter. The dissolving residue of a solvent defined herein is calculated as follows. 1g of toner is uniformly dissolved or dispersed in each 100mL solvent of THF, ethyl acetate and chloroform. The solution or dispersion solution is press filtered and a filtrate is dried and quantitated. The ratio of an insoluble substance to an organic solvent in the toner is calculated from the quantitated value and defined as the dissolving residue of a solvent.

The toner of the present invention can be used in the one-component development process, which is one of the image forming processes. The one-component development process is the process comprising the steps of providing a latent image support member with the thinned toner, and developing the latent images. The toner is usually thinned with a device wherein a toner carrying material, a toner layer thickness controlling material and a toner supply auxiliary material are equipped; and the toner supply auxiliary material and the toner carrying material, and the toner layer thickness controlling material and the toner carrying material abut each other.

The case in which the toner of the present invention is used in the two-component development process is further illustrated as follows. The two-component development process is the process wherein a toner and a carrier (those having roles as a charge provider and a toner carrying material) are used. The above magnetic materials or glass beads are used as a carrier. Developers (toner and a carrier) generate a specific charge amount by being stirred by a stirring material, and they are carried to a developing part by a magnet roller or the like. On the magnet roller, the developers are kept on the surface of the roller by magnetic force, and they form a magnetic brush whose layer is controlled to a suitable height by a developer control plate or the like. The developers move on the development roller as the roller rotates, and contact with an electrostatic latent image support member or face against it in a specific distance and in the noncontact condition to develop and visualize latent images. When developing images in the noncontact condition, a toner can usually obtain the driving force of flying the space of a specific distance by generating a direct electric field between developers and a latent image support member. However, in order to develop clearer images, it is possible to apply the method of superimposing alternating current.

Further, the charge control agent of the present invention is suitable for a charge control agent (a charge enhancer) in coating compounds for coating electrostatic powders. Namely, coating compounds for coating electrostatic powders using said charge enhancer are excellent in environment resistance and preservation stability, and particularly thermal stability and durability. Besides, the coating efficiency thereof reaches 100% and, therefore, it is possible to form thick film without coating defect.

### Example 1

Next, Examples will further illustrate the present invention. They only explain the present invention and do not particularly limit the invention. In examples, "part" means "part by weight".

The purity of the cyclic phenol sulfide of the formula (1) used in the present invention, relative proportions thereof and the like were analyzed by a high performance liquid chromatography (hereinafter referred to as HPLC). The purification of these compounds was conducted by column chromatography, adsorptive purification with silica gel, activated charcoal, activated earth and the like, recrystallization with a solvent, crystallization method, or the like. The identification of the compounds was conducted by NMR analysis.

25.0g (29.4mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 200mL of dimethylformamide (hereinafter referred to as DMF); and 32.6g (235.6mmol) of potassium carbonate were poured in a 500mL four-neck flask with a mixer, a cooling tube and a thermometer. 66.9g (471.1mmol) of iodomethane was added dropwise thereto under room temperature. Then, the reaction mixture was heated up to 60°C and stirred for 8 hours. After letting the mixture stand to cool to room temperature, precipitated crystals were collected by filtration. The obtained crude crystals were washed by dispersion with DMF three times, and washed by dispersion with ion-exchange water three times. Then, the crystals were dried under reduced pressure at 50°C overnight to obtain 25.11g (yield 94.4%) of a cyclic tetramer wherein, in the formula (1), R1 is a methyl group, R2 is a tert-butyl group, m is 4, and n is 2 as pale yellow crystals.

The structure of the obtained pale yellow crystals was identified using NMR. As a result, 56 following hydrogen signals were detected in 1H-NMR(CDCl₃): δ (ppm) = 1.30(36H), 3.97(12H), 8.21(8H).

Further, the result of the HPLC analysis indicated the peak area ratio of 96.3% as the purity of the crystals.

### Example 2

3.4g (4.0mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 80mL of DMF; and 2.2g (16.0mmol) of potassium carbonate were poured in a 200mL four-neck flask with a mixer, a cooling tube and a thermometer. 8.2g (48.2mmol) of 1-iodopropane was added dropwise thereto under room temperature. Then, the reaction mixture was heated up to 60°C and stirred for 8 hours. After letting the mixture stand to cool to room temperature, precipitated crystals were collected by filtration. The obtained crude crystals were washed by dispersion with DMF three times, and washed by dispersion with ion-exchange water three times. Then, the crystals were dissolved in chloroform, and the insoluble part thereof was filtered out. Then, the crystals obtained by concentration with an evaporator were dried under reduced pressure at 50°C overnight to obtain 2.60g (yield 63.9%) of a cyclic tetramer wherein, in the formula (1), R1 is a n-propyl group, R2 is a tert-butyl group, m is 4, and n is 2 as white crystals.

The structure of the obtained white crystals was identified using NMR. As a result, 72 following hydrogen signals were detected in 1H-NMR(CDCl₃): δ (ppm) = 0.66(12H), 1.06(8H), 1.36(36H), 4.19(8H), 8.38(8H).

### Example 3

6.8g (8.0mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 150mL of DMF; and 4.4g (32.0mmol) of potassium carbonate were poured in a 500mL four-neck flask with a mixer, a cooling tube and a thermometer. 16.9g (48.0mmol) of 1-iodohexadecane was added dropwise thereto under room temperature. Then, the reaction mixture was heated up to 60°C and stirred for 8 hours. After letting the mixture stand to cool to room temperature, precipitated crystals- were collected by filtration. The obtained crude crystals were washed by dispersion with DMF three times, and washed by dispersion with ion-exchange water three times. Then, the crystals were dissolved in chloroform, and the insoluble part thereof was filtered out. Then, the crystals obtained by concentration with an evaporator were dried under reduced pressure at 50°C overnight to obtain 7.68g (yield 55.0%) of a cyclic tetramer wherein, in the formula (1), R1 is a n-hexadecyl group, R2 is a tert-butyl group, m is 4, and n is 2 as white crystals.

The structure of the obtained white crystals was identified using NMR. As a result, 176 following hydrogen signals were detected in 1H-NMR(CDCl₃): δ (ppm) = 0.88(12H), 1.27(112H), 1.36(36H), 4.27(8H), 8.34(8H).

### Example 4

6.8g (8.0mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 150mL of DMF; and 4.4g (32.0mmol) of potassium carbonate were poured in a 500mL four-neck flask with a mixer, a cooling tube and a thermometer. 6.1g (48.0mmol of chlorinated benzyl was added dropwise thereto under room temperature. Then, the reaction mixture was heated up to 100°C and stirred for 8 hours. After letting the mixture stand to cool to room temperature, precipitated crystals were collected by filtration. The obtained crude crystals were washed by dispersion with DMF three times, and washed by dispersion with ion-exchange water three times. Then, the crystals were dissolved in chloroform, and the insoluble part thereof was filtered out. Then, the crystals obtained by concentration with an evaporator were dried under reduced pressure at 50°C overnight to obtain 2.07g (yield 14.2%) of a cyclic tetramer wherein, in the formula (1), R1 is a benzyl group, R2 is a tert-butyl group, m is 4, and n is 2 as white crystals.

The structure of the obtained white crystals was identified using NMR. As a result, 72 following hydrogen signals were detected in 1H-NMR(CDCIs): δ (ppm) = 0.83(36H), 5.34(8H), 7.35(12H), 7.74(8H), 8.24(8H).

### Example 5

5.5g (6.5mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 55mL of DMF; and 7.2g (52.1mmol) of potassium carbonate were poured in a 100mL four-neck flask with a mixer, a cooling tube and a thermometer. 25.0g (104.1mmol) of 1-iodo-n-octane was added dropwise thereto under room temperature. Then, the reaction mixture was heated up to 70°C and stirred for 3 hours. After letting the mixture stand to cool to room temperature, precipitated crystals were collected by filtration. The obtained crude crystals were washed by dispersion with DMF, and washed by dispersion with ion-exchange water twice. The crystals were further washed by dispersion with a dilute sulfuric acid (pH = 1) and methanol respectively, and dried under reduced pressure to obtain 4.17g (yield 49.6%) of a cyclic tetramer wherein, in the formula (1), R1 is a n-octyl group, R2 is a tert-butyl group, m is 4, and n is 2 as white crystals.

The structure of the obtained white crystals was identified using NMR. As a result, 120 following hydrogen signals were detected in 1H-NMR(CDCb): δ (ppm) = 0.90(12H), 1.12-1.42(92H), 4.24-4.26(8H), 8.34(8H).

### Example 6

6.8g (8.0mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 150mL of DMF; and 4.4g (32.0mmol) of potassium carbonate were poured in a 300mL four-neck flask with a mixer, a cooling tube and a thermometer. 6.1g (48.0mmol) of benzyl chloride was added thereto under room temperature. Then, the reaction mixture was heated up to 100°C and stirred for 8 hours. After letting the mixture stand to cool to room temperature, precipitated crystals were collected by filtration and repeatedly washed by dispersion with DMF Thus obtained crude crystals were dissolved in chloroform, and the insoluble part thereof was filtered out. Then, the crystals were concentrated under reduced pressure and further dried under reduced pressure at 50°Cto obtain 2.07g (yield 14.2%) of a cyclic tetramer wherein, in the formula (1), R1 is a benzyl group, R2 is a tert-butyl group, m is 4, and n is 2 as white crystals.

The structure of the obtained white crystals was identified using NMR. As a result, 72 following hydrogen signals were detected in 1H-NMR(CDCl₃): δ (ppm) = 0.83(36H), 5.34(8H), 7.35(12H), 7.74(8H), 8.24(8H).

### Example 7

12.74g (15.0mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 75mL of DMF; 16.59g (120.0mmol) of potassium carbonate; and 1.25g (7.5mmol) of potassium iodine were poured in a 300mL four-neck flask with a mixer, a cooling tube and a thermometer. 22.69g (240.0mmol) of 1-chloro-2-methoxyethane was added dropwise thereto under room temperature. The reaction mixture was heated up to 90°C and stirred for 2 hours, and then heated up to 110°C and stirred for 9 hours. 5.67g (60.0mmol) of 1-chloro-2-methoxyethane was further added dropwise thereto, and stirred at 110°C for 5 hours. After letting the mixture stand to cool to room temperature, precipitated crystals were collected by filtration. The obtained crude crystals were repeatedly washed by dispersion with DMF, and then repeatedly washed by dispersion with ion-exchange water. The crystals were further repeatedly washed by dispersion with a dilute sulfuric acid (pH = 1) and methanol respectively. Then, the crystals were dried under reduced pressure at 100°C for 3 hours to obtain 13.60g (yield 83.8%) of a cyclic tetramer wherein, in the formula (1), R1 is a 2-methoxyethyl group, R2 is a tert-butyl group, m is 4, and n is 2 as white crystals.

The structure of the obtained white crystals was observed using NMR.

### Example 8

20.0g (23.6mmol) of 4-(tert-butyl) sulfonyl calix[4]arene corresponding to a cyclic tetramer wherein, in the formula (1), R1 is a hydrogen atom, R2 is a tert-butyl group, m is 4, and n is 2; 200mL of DMF; and 16.4g (118.7mmol) of potassium carbonate were poured in a 300mL four-neck flask with a mixer, a cooling tube and a thermometer. 32.0g (191.6mmol) of ethyl bromoacetate was added dropwise thereto under room temperature. The reaction mixture was heated up to 60°C and stirred for 11 hours. After letting the mixture stand to cool to room temperature, precipitated crystals were filtered out. Then, 250mL of ion-exchange water and 250mL of chloroform were added thereto and stirred to separate an organic layer. Thus obtained organic layer was dehydrated with anhydrous magnesium sulfate and concentrated under reduced pressure to obtain 4.30g (yield 21.4%) of a cyclic tetramer wherein, in the formula (1), R1 is an ethoxycarbonylmethyl group, R2 is a tert-butyl group, m is 4, and n is 2 as white crystals.

The structure of the obtained white crystals was observed using NMR.

### Example 9

123.79g of 4-(1,1,3,3-tetramethylbutyl)phenol, 38.48g of sulfur and 12.00g of sodium hydroxide were poured in a 1L four-neck flask with a mixer, a cooling tube, a thermometer and a gas-introducing tube. 371.4g of diphenyl ether was added thereto and stirred in the current of nitrogen gas while keeping it at 130°C. The reaction was conducted for 1 hour with removing water and hydrogen sulfide each of which was generated in the reaction. After heating it up to 240°C, the reaction was further conducted for 15.5 hours with removing water and hydrogen sulfide each of which was generated in the reaction. The reaction mixture was cooled down to room temperature, and 150mL of a mixed solvent of isopropyl alcohol/water (88/12, v/v) and 60mL of a 20% sulfuric acid were added thereto and stirred. Precipitated crystals were collected by filtration and washed by dispersion with a mixed solvent of isopropyl alcohol/water (88/12, v/v) twice and then with ion-exchange water twice. The crystals were further washed by dispersion with a mixed solvent of isopropyl alcohol/water (88/12, v/v) and dried under reduced pressure to obtain 59.13g (yield 41.7%) of a cyclic tetramer wherein, in the formula (1), R1 is a hydrogen atom, R2 is a 1,1,3,3-tetramethylbutyl group, m is 4, and n is 0 as beige crystals.

113.46g of the cyclic tetramer obtained by repeating the above reaction wherein, in the formula (1), R1 is a hydrogen atom, R2 is a 1,1,3,3-tetramethylbutyl group, m is 4, and n is 0; 340.4g of an acetic acid; 8.16g of sodium acetate trihydrate; 22.7g of toluene; and 7.92g of sodium tungstate dehydrate were poured in a 1L four-neck flask with a mixer, a cooling tube and a thermometer. 186.6g of a 30% hydrogen peroxide water was added dropwise thereto for 4.5 hours with controlling the solution temperature to 60°C, and the reaction mixture was stirred at 60°C for 11 hours. 93.3g of a 30% hydrogen peroxide water was further added dropwise thereto and stirred at 60°C for 8 hours. 15.6g of a concentrated hydrochloric acid was added dropwise thereto at 60°C and further stirred for 1 hour. After letting the mixture stand to cool to room temperature, precipitated crystals were collected by filtration. The obtained crude crystals were washed by dispersion with ion-exchange water twice, and then washed by dispersion with a mixed solvent of methanol/water (1/1, v/v). Then, the crystals were dried under reduced pressure to obtain 121.19g (yield 94.1%) of a cyclic tetramer wherein, in the formula (1), R1 is a hydrogen atom, R2 is a 1,1,3,3-tetramethylbutyl group, m is 4, and n is 2 as white crystals.

64.41g (60.0mmol) of thus obtained cyclic tetramer wherein, in the formula (1), R1 is a hydrogen atom, R2 is a 1,1,3,3-tetramethylbutyl group, m is 4, and n is 2; 644.09mL of DMF; and 66.34g (480.0mmol) of potassium carbonate were poured in a 1L four-neck flask with a mixer, a cooling tube and a thermometer. 136.26g (960.0mmol) of iodomethane was added dropwise thereto under room temperature. Then, the reaction mixture was heated up to 70°C and stirred for 3 hours. After letting the mixture stand to cool to room temperature, precipitated crystals were collected by filtration. The obtained crude crystals were repeatedly washed by dispersion with DMF, a dilute sulfuric acid (pH = 1), ion-exchange water, and a mixed solvent of isopropyl alcohol/water (88/12, v/v) respectively. Then, the crystals were dried under reduced pressure to obtain 64.00g (yield 94.4%) of a cyclic tetramer wherein, in the formula (1), R1 is a methyl group, R2 is a 1,1,3,3-tetramethylbutyl group, m is 4, and n is 2 as pale cream-colored crystals.

### Example 10

### [Preparation of a resin dispersion solution]

80 parts of polyester resin (DIACRON ER-561 produced by Mitsubishi Rayon Co., Ltd.), 320 parts of ethyl acetate and 32 parts of isopropyl alcohol were mixed, and appropriate quantities of 0.1mass% ammonia water were added dropwise to the mixture to conduct phase-transfer emulsification with stirring it at 5000 to 10000 rpm using a homogenizer (Awa-less mixer NGM-0.5TB produced by Beryu Co., Ltd.). Then, the pressure thereof was reduced with an evaporator to remove the solvent, and a resin dispersion solution was obtained. The volume average particle diameter of resin particles in this dispersion solution was 0.2 µ m (The resin particle concentration was adjusted with ion-exchange water to become 20mass%).

### [Preparation of a dispersion solution of a charge control agent]

0.2 part of sodium dodecylbenzenesulfonate, 0.2 part of Sorbon T-20 (produced by TOHO Chemical Industry Co., Ltd.) and 17.6 parts of ion-exchange water were mixed and dissolved. 2.0 parts of the cyclic tetramer synthesized in Example 1 wherein, in the formula (1), R1 is a methyl group, R2 is a tert-butyl group, m is 4, and n is 2; and zirconia beads (particle diameter of beads: 0.65mm φ, 15mL equivalent) were added thereto and dispersed for 3 hours with a paint conditioner (Red Devil No. 5400-5L produced by UNION N.J. (USA)). The zirconia beads were removed using a sieve, and the mixture was adjusted by ion-exchange water to prepare a 10mass% dispersion solution of a charge control agent. In this dispersion solution of a charge control agent, the volume average particle diameter of the cyclic tetramer synthesized in Example 1 wherein, in the formula (1), R1 is a methyl group, R2 is a tert-butyl group, m is 4, and n is 2 was 0.34µm.

### [Preparation of a polymerized toner]

125 parts of the resin dispersion solution, 1.0 part of a 20 mass% aqueous solution of sodium dodecylbenzenesulfonate and 125 parts of ion-exchange water were poured in a reaction container with a thermometer, pH meter and a mixer, and stirred at 150 rpm for 30 minutes with controlling the solution temperature to 30°C. A 1 mass% nitric acid aqueous solution was added thereto to adjust pH to 3.0, and the mixture was further stirred for 5 minutes. With dispersing it with a homogenizer (ULTRA-TURRAX T-25 produced by IKA Japan), 0.125 part of polyaluminum chloride was added thereto. After heating the solution up to 50°C, the mixture was stirred for 30 minutes. 62.5 parts of the resin dispersion solution and 4.0 parts of the dispersion solution of a charge control agent were added thereto. A 1 mass% nitric acid aqueous solution was further added thereto to adjust pH to 3.0, and the mixture was further stirred for 30 minutes. With stirring the mixture at 400 to 700 rpm using a mixer, 8.0 parts of a 5 mass% aqueous solution of sodium hydroxide was added thereto, and stirring was continued until the volume average particle diameter of the toner becomes 9.5µm. After heating the solution up to 75°C, the mixture was further stirred for 2 hours. After confirming that the volume average particle diameter becomes 6.0µm and that the particle form becomes spherical, the mixture was rapidly cooled down with ice water. Precipitates were collected by filtration and washed by dispersion with ion-exchange water. The washing by dispersion was repeated until the electrical conductivity of a filtrate after the dispersion becomes 20 µ S/cm or less. Then, the precipitates were dried by a dryer at 40°C to obtain toner particles.

The obtained toner was sieved by a 166 mesh sieve (sieve opening 90µ m) to obtain a toner for evaluation.

### [Evaluation]

2 parts of the obtained toner for evaluation and 100 parts of a non-coat ferrite carrier (F-150 produced by Powdertech Co., Ltd.) were mixed and shaken to charge the toner negatively. Then, the saturated charge amount of the toner was measured with a blow-off powder charge amount measurement device at 25°C and at 50% humidity. Also, in the case of mixing the toner with a silicone-coated ferrite carrier (F96-150 produced by Powdertech Co., Ltd.), the same evaluation was conducted. The results are shown in Table 1.

### Example 11

A toner was prepared by the same condition as that of Example 10 except that the dispersion solution of a charge control agent was prepared using the cyclic tetramer synthesized in Example 6 wherein, in the formula (1), R1 is a benzyl group, R2 is a tert-butyl group, m is 4, and n is 2 instead of the cyclic tetramer synthesized in Example 1 wherein, in the formula (1), R1 is a methyl group, R2 is a tert-butyl group, m is 4, and n is 2. Then, the saturated charge amount of the toner was measured.

The results are shown in Table 1.

### Example 12

A toner was prepared by the same condition as that of Example 10 except that the dispersion solution of a charge control agent was prepared using the cyclic tetramer synthesized in Example 9 wherein, in the formula (1), R1 is a methyl group, R2 is a 1,1,3,3-tetramethylbutyl group, m is 4, and n is 2 instead of the cyclic tetramer synthesized in Example 1 wherein, in the formula (1), R1 is a methyl group, R2 is a tert-butyl group, m is 4, and n is 2. Then, the saturated charge amount of the toner was measured.

The results are shown in Table 1.

### [Comparative Example 1]

For comparison, a toner was prepared by the same condition as that of Example 10 except that the step of adding the dispersion solution of a charge control agent was omitted. Then, the saturated charge amount of the toner was measured.

The results are shown in Table 1.

### [Comparative Example 2]

For comparison, a toner was prepared by the same condition as that of Example 10 except that the dispersion solution of a charge control agent was prepared using 4-(tert-butyl) sulfonyl calix[4]arene corresponding to a cyclic tetramer wherein, in the formula (1), R1 is a hydrogen atom, R2 is a tert-butyl group, m is 4, and n is 2 instead of the cyclic tetramer synthesized in Example 1 wherein, in the formula (1), R1 is a methyl group, R2 is a tert-butyl group, m is 4, and n is 2. Then, the saturated charge amount of the toner was measured.

The results are shown in Table 1.

**Table 1**

| | Carrier F-150 | Carrier F96-150 |
|---|---|---|
| | Charge amount (µc/g) | Charge amount (µc/g) |
| Example 10 | -60.78 | -27.70 |
| Example 11 | -71.59 | -24.05 |
| Example 12 | -61.82 | -37.56 |
| Comp.Exam.1 | -54.13 | -20.46 |
| Comp.Exam.2 | -35.29 | -12.30 |

As is clear from the results of Table 1, a polymerized toner comprising a cyclic phenol sulfide(s) of the formula (1) of the present invention as an active ingredient has excellent charging performance.

Namely, it is possible to provide a polymerized toner with high charging performance by using a charge control agent comprising a cyclic phenol sulfide(s) of the formula (1) of the present invention as an active ingredient.

The cyclic phenol sulfides of the formula (1) of the present invention have excellent charging performance, and charge control agents containing said compound(s) clearly have higher charging performance and excellent environmental stability than conventional charge control agents. Further, since they are completely colorless, they are most useful for color toners and particularly for polymerized toners. Besides, they do not comprise heavy metals such as chromium compounds, which are concern for the environmental problem, and thus, it is possible to provide extremely useful toners.

## Claims

1. A polymerized toner comprising one or more kinds of a cyclic phenol sulfide(s) of the following formula (1): wherein R1 is a substituted or unsubstituted and straight or branched alkyl group having 1 to 20 carbon atoms, a substituted or unsubstituted aromatic hydrocarbon group, or a substituted or unsubstituted condensed polycyclic aromatic group; R2 is a substituted or unsubstituted and straight or branched alkyl group having 1 to 20 carbon atoms, a substituted or unsubstituted aromatic hydrocarbon group, a substituted or unsubstituted aromatic heterocyclic group, or a substituted or unsubstituted condensed polycyclic aromatic group; m is an integer from 4 to 9; and n is an integer of 0, 1 or 2.

2. The polymerized toner according to claim 1, wherein, in the formula (1), R2 is a substituted or unsubstituted aromatic hydrocarbon group, a substituted or unsubstituted aromatic heterocyclic group, or a substituted or unsubstituted condensed polycyclic aromatic group.

3. The polymerized toner according to claim 1 or 2, wherein, in the formula (1), R2 is an aromatic hydrocarbon group with a substituent(s), a substituted or unsubstituted aromatic heterocyclic group, or a condensed polycyclic aromatic group with a substituent(s).

4. The polymerized toner according to any one of claims 1 to 3, wherein, in the formula (1), R2 is a substituted or unsubstituted aromatic heterocyclic group.

5. The polymerized toner according to claim 1, wherein, in the formula (1), R1 is an alkyl group or a phenylalkyl group.

6. The polymerized toner according to claim 5, wherein, in the formula (1), R2 is a branched alkyl group.

7. The polymerized toner according to any one of claims 1 to 6 comprising one or more kinds of the cyclic phenol sulfide(s) of the formula (1), wherein m is 4 or 8; and n is 2.

8. The polymerized toner according to any one of claims 1 to 7 comprising a binder resin, wherein the binder resin is selected from the group consisting of polyester resins, (meth)acrylic resins, polyol resins, phenol resins, silicone resins, polyurethane resins, polyamide resins, furan resins, epoxy resins, xylene resins, terpene resins, coumarone-indene resins, polycarbonate resins and petroleum resins.

9. The polymerized toner according to claim 8, wherein the binder resin is a polyester resin.
